

# United States Patent [19]

Saitoh et al.

[11] Patent Number: 4,598,032

[45] Date of Patent: Jul. 1, 1986

[54] PHOTOCOCONDUCTIVE MEMBER WITH A-SI; A-(SI/GE) AND A-(SI/C) LAYERS

[75] Inventors: Keishi Saitoh, Ibaraki; Yukihiko Ohnuki, Kawasaki; Shigeru Ohno, Yokohama, all of Japan

[73] Assignee: Canon Kabushiki Kaisha, Tokyo, Japan

[21] Appl. No.: 686,939

[22] Filed: Dec. 27, 1984

[30] Foreign Application Priority Data

Dec. 29, 1983 [JP] Japan 58-250269  
Dec. 30, 1983 [JP] Japan 58-246523  
Dec. 31, 1983 [JP] Japan 58-246735

[51] Int. Cl. 4 G03G 5/082

[52] U.S. Cl. 430/58; 430/84; 430/85; 430/95

[58] Field of Search 430/58, 84, 85, 95

[56]

References Cited

U.S. PATENT DOCUMENTS

4,451,546 5/1984 Kawarzura et al. .... 430/69  
4,495,262 1/1985 Matsuzaki et al. .... 430/58

Primary Examiner—John L. Goodrow

Attorney, Agent, or Firm—Fitzpatrick, Cella, Harper & Scinto

[57] ABSTRACT

A photoconductive member having a substrate for photoconductive member and a light-receiving layer having photoconductivity provided on said substrate is prepared in which the light-receiving layer comprises from the side of said substrate a first layer (I) constituted of an amorphous material containing silicon atoms, a second layer (II) constituted of an amorphous material containing silicon atoms and germanium atoms and a third layer (III) constituted of an amorphous material containing silicon atoms and carbon atoms, and the germanium atoms contained in said second layer (II) being distributed ununiformly in the layer thickness direction of said layer.

26 Claims, 25 Drawing Figures

FIG. 1



FIG. 2



FIG. 3



FIG. 4



FIG. 5



FIG. 8



FIG. 6



FIG. 9



FIG. 7



FIG. 10



FIG. 11



FIG. 12



FIG. 13



FIG. 14A



FIG. 14B



FIG. 15



FIG. 16



FIG. 17





FIG. 19



FIG. 20



FIG. 21



FIG. 22



FIG. 23



FIG. 24



**PHOTOCONDUCTIVE MEMBER WITH A-Si;  
A-(Si/Ge) AND A-(Si/C LAYERS**

**BACKGROUND OF THE INVENTION**

**1. Field of the Invention**

This invention relates to a photoconductive member having sensitivity to electromagnetic waves such as light (herein used in a broad sense, including ultraviolet rays, visible light, infrared rays, X-rays, gamma-rays etc.).

**2. Description of the Prior Art**

Photoconductive materials, which constitute photoconductive layer in solid stage image pick-up devices, image forming members for electrophotography in the field of image formation, or manuscript reading devices and the like, are required to have a high sensitivity, a high SN ratio (Photocurrent ( $I_p$ )/dark current ( $I_d$ )), absorption spectral characteristics matching to those of electromagnetic waves to be irradiated, a rapid response to light, a desired dark resistance value as well as no danger to human bodies during usage. Further, in a solid state image pick-up device, it is also required that the residual image should easily be treated within a predetermined time. Particularly, in case of an image forming member for electrophotography to be assembled in an electrophotographic device to be used in an office as office apparatus, the aforesaid safety characteristic is very important.

From the standpoint as mentioned above, amorphous silicon (hereinafter referred to as a-Si) has recently attracted attention as a photoconductive material. For example, German OLS Nos. 2746967 and 2855718 disclose applications of a-Si for use in image forming members for electrophotography, and German OLS Nos. 2933411 discloses an application of a-Si for use in a photoconverting reading device.

However, under the present situation, the photoconductive members of the prior art having light-receiving layers constituted of a-Si are further required to be improved in a balance of overall characteristics including electrical, optical and photoconductive characteristics such as dark resistance value, photosensitivity and response to light, etc., and environmental characteristics during use such as humidity resistance, and further stability with lapse of time.

For instance, when the above light-receiving member is applied in an image forming member for electrophotography, residual potential is frequently observed to remain during use thereof if improvements to higher photosensitivity and higher dark resistance are scheduled to be effected at the same time. When such a photoconductive member is repeatedly used for a long time, there will be caused various inconveniences. For example, accumulation of fatigue occurs by repeated uses to give rise to so called ghost phenomenon wherein residual images are formed, or response characteristic is gradually lowered when it is used repeatedly at high speed.

Further, a-Si has a relatively smaller coefficient of absorption of the light on the longer wavelength side in the visible light region as compared with that on the shorter wavelength side. Accordingly, in matching to the semiconductor laser conventionally applied at the present time, the light on the longer wavelength side cannot effectively utilized, when employing a halogen

lamp or a fluorescent lamp as the light source. Thus, various points remain to be improved.

On the other hand, when the light irradiated is not sufficiently absorbed in the photoconductive layer, but the amount of the light reaching the substrate (or support) is increased, interference due to multiple reflection may occur in the photoconductive layer to become a source for "unfocused" image, in the case when the substrate itself has a high reflectance against the light permeated through the photoconductive layer.

This effect will be increased, if the irradiated spot is made smaller for purpose of enhancing resolution, thus posing a great problem in the case of using a semiconductor laser as the light source.

Further, a-Si materials may contain as constituent atoms hydrogen atoms or halogen atoms such as fluorine atoms, chlorine atoms, etc. for improving their electrical, photoconductive characteristics, boron atoms, phosphorus atoms, etc. for controlling the electroconduction type as well as other atoms for improving other characteristics. Depending on the manner in which these constituent atoms are contained, there may sometimes be caused problems with respect to electrical or photoconductive characteristics of the layer formed.

That is, for example, in many cases, the life of the photocarriers generated by light irradiation on the photoconductive layer formed is insufficient, or at the dark portion, the charges injected from the substrate side cannot sufficiently be impeded.

Accordingly, while attempting to improve the characteristics of a-Si material per se on one hand, it is also required to make efforts to overcome all the problems as mentioned above in designing of the light-receiving member on the other hand.

**SUMMARY OF THE INVENTION**

The present invention has been achieved to solve the above-mentioned drawbacks of photoconductive member of the prior art after comprehensive studies in view of the applicability of a-Si to an electrophotographic image-forming member as well as to a photoconductive member for a solid-state image pick-up device, a read-out device, etc. The photoconductive member having a specific layer structure has been found excellent which is constituted of (A) an amorphous material having silicon as a matrix, especially an amorphous material having a silicon atom (Si) matrix and containing at least one of hydrogen atoms (H) or halogen atoms (X), i.e. so-called hydrogenated amorphous silicon or halogenated amorphous silicon (hereinafter collectively referred to as "a-Si(H, X)") and (B) an amorphous material having silicon atoms (Si) and germanium atoms (Ge) as a matrix, especially an amorphous material having said atoms as a matrix and containing at least one of hydrogen atoms (H) or halogen atoms, i.e. so-called hydrogenated amorphous silicon germanium, halogenated amorphous silicon germanium, or halogen-containing hydrogenated amorphous silicon germanium (hereinafter collectively referred to as "a-SiGe(H, X)"). The photoconductive member not only has superior practical characteristics, but also surpasses photoconductive members of the prior art in every respect, especially has excellent characteristics in the use for electrophotography and in the long wavelength region.

A primary object of the present invention is to provide a photoconductive member having electrical, optical and photoconductive characteristics which are constantly stable and all-environment type with virtually

no dependence on the environments under use, which member has excellent photosensitivity characteristics in long wavelength side and is markedly excellent in light fatigue resistance and in durability without causing deterioration phenomenon when used repeatedly, exhibiting no or substantially no residual potential observed.

Another object of the present invention is to provide a photoconductive member which is high in photosensitivity throughout the whole visible light region, particularly excellent in matching to a semiconductor laser and also rapid in light response.

Still another object of the present invention is to provide a photoconductive member having sufficient chart retentivity during charging treatment for formation of electrostatic images to the extent such that a conventional electrophotographic method can be very effectively applied when it is provided for use as an image forming member for electrophotography.

Further, still another object of the present invention is to provide a photoconductive member for electrophotography, which can easily provide an image of high quality which is high in density, clear in halftone and high in resolution without formation of image defect or image flow.

Still another object of the present invention is to provide a photoconductive member, capable of giving sufficiently high dark resistance and sufficient acceptance potential, and also to improve productivity through improvement of adhesion between respective layers.

Still another object of the present invention is to provide a photoconductive member having high photosensitivity and high SN ratio characteristic.

According to the present invention, there is provided a photoconductive member comprising a substrate for photoconductive member and a light-receiving layer exhibiting photoconductivity, said light-receiving layer having a layer constitution in which a first layer (I) comprising an amorphous material containing silicon atoms, a second layer (II) comprising an amorphous material containing silicon atoms and germanium atoms and a third layer (III) comprising an amorphous material containing silicon atoms and carbon atoms are successively provided from the substrate side, and the germanium atoms contained in said second layer (II) being distributed ununiformly in the direction of the thickness said layer.

It is desirable that hydrogen atoms and/or halogen atoms should be contained in at least one of the aforesaid first layer (I) and the aforesaid second layer (II) and it is also preferred that a substance for controlling conductivity should be contained in at least one of the aforesaid first layer (I) and the aforesaid second layer (II).

Further, if desired, at least one of oxygen atoms and nitrogen atoms may be contained in at least one of the aforesaid first layer (I) and the aforesaid second layer (II).

The photoconductive member of the present invention designed to have such a layer constitution as mentioned above can solve all of the various problems as mentioned above and exhibit very excellent electrical, optical, photoconductive characteristics, dielectric strength and use environment characteristics.

In particular, the photoconductive member of the present invention is free from any influence from residual potential on image formation when applied for an

image forming member for electrophotography, with its electrical characteristics being stable with high sensitivity, having a high SN ratio as well as excellent light fatigue resistance and excellent repeated use characteristic and being capable of providing images of high quality of high density, clear halftone and high resolution repeatedly and stably.

Further, the photoconductive member of the present invention is high in photosensitivity over all the visible light region, particularly excellent in matching to semiconductor laser, excellent in interference inhibition and rapid in response to light.

#### BRIEF DESCRIPTION OF THE DRAWINGS

FIG. 1 shows a schematic sectional view for illustration of the layer constitution of the photoconductive member according to the present invention;

FIGS. 2 through 13 each show a schematic illustration of the depth profile of germanium atoms in the second layer (II) in the photoconductive member of the present invention;

FIGS. 14A, 14B and FIG. 16 each show schematically the concentration distribution of boron atoms in the light-receiving layer in Examples of the photoconductive member of the present invention;

FIGS. 15, 17, 21 and 24 each shows schematically the concentration distribution of germanium atoms in the second layer (II) of the present invention;

FIG. 18 is a drawing showing the preparation device of the photoconductive member according to the flow discharge decomposition method;

FIGS. 19 and 20 each show schematically the concentration distribution of oxygen atoms in the light-receiving layer in Examples of the photoconductive member of the present invention; and

FIGS. 22 and 23 each show schematically the concentration distribution of nitrogen atoms in the light-receiving layer in Examples of the photoconductive members of the present invention.

#### DETAILED DESCRIPTION OF THE PREFERRED EMBODIMENT

Referring now to the drawings, the photoconductive member of the present invention is to be described in detail.

FIG. 1 shows schematically the layer constitution of the photoconductive member of the present invention.

The photoconductive member 100 of the present invention has a light-receiving layer 102 having sufficient volume resistance and photoconductivity on a substrate 101 for photoconductive member. The light-receiving layer 102 is constituted, from the aforesaid substrate side, of a first layer (I) 103 comprising a-Si(H, X), a second layer (II) 104 comprising a-SiGe(H, X) and a third layer (III) 105 comprising a-SiC(H, X). Although photoconductivity may be possessed by either one of the first layer (I) and the second layer (II), it is anyway necessary to design the layer so that the layer which the incident light reaches may have photoconductivity. Also, in this case, it is desirable that both of the first layer (I) and the second layer (II) should have photoconductivity to the light having respectively desirable wavelength spectra, and that the layer should be designed so as to be able to generate sufficient amount of photocarriers.

In the photoconductive member of the present invention, by incorporating a substance (C) for controlling conductivity in at least one of the first layer (I) and the

second layer (II), the conductivity of the layer to be contained can be controlled as desired. Said substance (C) may be contained in both or each of the first layer (I) and the second layer (II) either uniformly or ununiformly in the layer thickness direction. Also, in the layer region (PN) where the substance (C) is contained, the substance (C) may be contained continuously, either uniformly or ununiformly in the layer thickness direction.

For example, when the second layer (II) is made thicker than the first layer (I), in order to employ the second layer (II) so as to have the function of a charge generating layer and a charge transporting layer, the substance (C) for controlling conductivity should desirably be contained in a distribution to be enriched on the substrate side. On the other hand, the substance (C) for controlling conductivity should desirably be contained in the second layer (II) so that it is more enriched on the interface between the first layer (I) and the second layer (II) or in the vicinity of the interface.

On the other hand, when the first layer (I) is made thicker than the second layer (II), in order to make the second layer (II) serve as a charge generating layer and the first layer (I) serve as a charge transporting layer, it is desirable that the substance (C) for controlling conductivity should be contained so as to be more enriched on the substrate side of the first layer (I).

Thus, in the present invention, by providing a layer region (PN) containing a substance (C) for controlling conductivity continuously in the layer thickness direction in at least one of the first layer (I) and the second layer (II), it is possible to effect improvement to higher sensitivity and higher dielectric strength.

As a substance (C) for controlling conductivity characteristics, there may be mentioned so called impurities in the field of semiconductors. In the present invention, there may be included p-type impurities giving p-type conductivity characteristics and n-type impurities giving n-type conductivity characteristics to Si or Ge constituting the layer region (PN). More specifically, there may be mentioned as p-type impurities atoms belonging to the group III of the periodic table (Group III atoms), such as B (boron), Al(aluminum), Ga(gallium), In(indium), Tl (thallium), etc., particularly preferably B and Ga. As n-type impurities, there may be included atoms belonging to the group V of the periodic table, such as P(phosphorus), As(arsenic), Sb(antimony), Bi(bismuth), etc., particularly preferably P and As.

In the present invention, the content of the substance (C) for controlling conductivity in the layer region (PN) provided in the light-receiving layer may be suitably be selected depending on the conductivity required for said layer region (PN), or when said layer region (PN) is provided in direct contact with the substrate, depending on the organic relationships such as the relation with the characteristics at the contact interface with the substrate, etc. Also, the content of the substance (C) for controlling conductivity is determined suitably with due considerations of the relationships with characteristics of other layer regions provided in direct contact with said layer region (PN) or the characteristics at the contacted interface with said other layer regions.

In the present invention, the content of the substance (C) for controlling conductivity contained in the layer region (PN) should preferably be 0.001 to  $5 \times 10^4$  atomic ppm, more preferably 0.5 to  $1 \times 10^4$  atomic ppm, most preferably  $1 - 5 \times 10^3$  atomic ppm.

In the present invention, by making the content of the substance (C) for controlling conductivity in the layer region (PN) preferably 30 atomic ppm or more, more preferably 50 atomic ppm or more, most preferably 100 atomic ppm or more, for example, in the case when said substance (C) to be incorporated is a p-type impurity as mentioned above, injection of electrons from the substrate side into the light-receiving layer can be effectively inhibited when the free surface of the light-receiving layer is subjected to the charging treatment to  $\oplus$  polarity. On the other hand, when the substance to be incorporated is a n-type impurity, injection of positive holes from the substrate side into the light-receiving layer can be effectively inhibited when the free surface of the light-receiving layer is subjected to the charging treatment to  $\ominus$  polarity.

In the case as mentioned above, the layer region (Z) which is the portion excluding the above layer region (PN) under the basic constitution of the present invention as described above may contain a substance for controlling conductivity of the other polarity, or a substance for controlling conductivity characteristics of the same polarity may be contained therein in an amount by far smaller than that practically contained in the layer region (PN).

In such a case, the content of the substance (C) for controlling conductivity contained in the above layer region (Z) can be determined adequately as desired depending on the polarity or the content of the substance contained in the layer region (PN), but it is preferably 0.001 to 1000 atomic ppm, more preferably 0.05 to 500 atomic ppm, most preferably 0.1 to 200 atomic ppm.

In the present invention, when the same kind of a substance for controlling conductivity is contained in the layer region (PN) and the layer region (Z), the content in the layer region (Z) should preferably be 30 atomic ppm or less. Being different from the cases as mentioned above, in the present invention, it is also possible to provide a layer region containing a substance for controlling conductivity having one polarity and a layer region containing a substance for controlling conductivity having the other polarity in direct contact with each other, thus providing a so called depletion layer at said contact region. In short, for example, a layer containing the aforesaid p-type impurity and a layer region containing the aforesaid n-type impurity are provided in the light-receiving layer in direct contact with each other to form the so called p-n junction, whereby a depletion layer can be provided.

In the present invention, illustrative of halogen atoms (X), which may optionally be incorporated in the first layer (I) are fluorine, chlorine, bromine and iodine, particularly preferably fluorine and chlorine.

In the present invention, formation of the first layer (I) constituted of a-Si(H, X) may be conducted according to the vacuum deposition method utilizing discharging phenomenon, such as glow discharge method, sputtering method or ion-plating method.

For example, for formation of the first layer (I) constituted of a-Si(H, X) according to the glow discharge method, the basic procedure comprises introducing a starting gas for Si supply capable of supplying silicon atoms (Si), and a starting gas for introduction of hydrogen atoms (H) and/or halogen atoms (X) into a deposition chamber which can be internally brought to a state of reduced pressure, and exciting glow discharge in said deposition chamber, thereby effecting layer formation.

of the first layer (I) constituted of a-Si(H, X) on the surface of a support placed at a predetermined position.

Alternatively, for formation according to the sputtering method, when carrying out sputtering by use of a target constituted of Si in an atmosphere of an inert gas such as Ar, He, etc. or a gas mixture based on these gases, a gas for introduction of hydrogen atoms (H) and/or halogen atoms (X) may be introduced into a deposition chamber for sputtering.

In the present invention, as the effective starting materials for the starting gases to be employed for formation of the first layer (I), the following compounds may be included.

First, the starting gas for supplying Si to be used in the present invention may include gaseous or gasifiable hydrogenated silicons (silanes) such as SiH<sub>4</sub>, Si<sub>2</sub>H<sub>6</sub>, Si<sub>3</sub>H<sub>8</sub>, Si<sub>4</sub>H<sub>10</sub> and others as effective materials. In particular, SiH<sub>4</sub> and Si<sub>2</sub>H<sub>6</sub> are preferred with respect to easy handling during layer formation and efficiency for supplying Si.

As the starting materials effectively used for supplying Si, in addition to hydrogenated silicon as mentioned above, there may be included silicon compounds containing halogen atoms (X), namely the so-called silane derivatives substituted with halogen atoms, including halogenated silicon such as SiF<sub>4</sub>, Si<sub>2</sub>F<sub>6</sub>, SiCl<sub>4</sub>, SiBr<sub>4</sub>, etc., as preferable ones. Further, halides containing hydrogen atom as one of the constituents, which are gaseous or gasifiable, such as halo-substituted hydrogenated silicon, including SiH<sub>2</sub>F<sub>2</sub>, SiH<sub>2</sub>I<sub>2</sub>, SiH<sub>2</sub>Cl<sub>2</sub>, SiHCl<sub>3</sub>, SiH<sub>2</sub>Br<sub>2</sub>, SiHBr<sub>3</sub>, etc. may also be mentioned as the effective starting materials for supplying Si for formation of the first layer (I).

Also, in the case of employing a silicon compound containing halogen atoms (X), X can be introduced together with Si in the layer formed by suitable choice of the layer formation conditions as mentioned above.

Effective starting materials to be used as the starting gases for introduction of halogen atoms (X) in formation of the first layer (I) in the present invention, there may be included, in addition to those as mentioned above, for example, halogen gases such as fluorine, chlorine, bromine and iodine; interhalogen compounds such as ClF, ClF<sub>3</sub>, BrF, BrF<sub>3</sub>, BrF<sub>5</sub>, IF<sub>3</sub>, IF<sub>7</sub>, ICl, IBr, etc.

In the present invention, when a layer region (ON) containing at least one of oxygen atoms and nitrogen atoms is provided in the desired layer region in the first layer (I), a starting material for introduction of oxygen atoms and/or nitrogen atoms may be used in combination while controlling its amount during formation of the first layer (I) by use of the above starting materials thereby incorporating oxygen atoms and/or nitrogen atoms in the layer formed.

The oxygen atoms or/and nitrogen atoms contained in the second layer (I) may be contained either throughout the whole region or only in a part of the region.

The distribution state C(ON) of oxygen atoms and/or nitrogen atoms may be either uniform or ununiform in the layer thickness direction of the first layer (I).

In the present invention, the layer region (ON) containing oxygen atoms and/or nitrogen atoms provided in the first layer (I) is provided so as to occupy the whole layer region of the first layer (I) when it is intended to improve photosensitivity and dark resistance, while it is provided so as to occupy the end portion layer region of the substrate and/or the second layer

(II) when it is intended to strengthen adhesion with the substrate and/or the second layer (II).

The content of oxygen atoms and/or nitrogen atoms to be contained in the layer region (ON) provided in such a first layer (I) can be selected suitably depending on the characteristics required for the layer region (ON) itself so as to accomplish the objects as mentioned above, the characteristics required at the contacted interface with the substrate or organic relationships with the characteristics possessed by other layer regions provided in direct contact with the layer region (ON), the characteristics required at the contacted interface with other layer regions, etc.

The content of oxygen atoms and/or nitrogen atoms in the layer region (ON), which may be determined suitably as desired depending on the characteristics of the photoconductive member to be formed, may be preferably 0.001 to 50 atomic %, more preferably 0.002 to 40 atomic %, most preferably 0.003 to 30 atomic %.

When the glow discharge method is applied for formation of the layer region (ON), the starting materials for introduction of oxygen atoms and/or nitrogen atoms are further added to those selected as desired from among the starting materials for formation of the first layer (I), as such starting materials for introduction of oxygen atoms and/or nitrogen atoms, there may be employed most of gaseous or gasified gasifiable substances having oxygen atoms and/or nitrogen atoms as constituent atoms.

As the starting materials effectively used for supplying oxygen atoms (O) for formation of the layer region (ON), there may be employed a starting gas containing O as constituent atoms or a starting gas containing O and H as constituent atoms, for example, oxygen (O<sub>2</sub>), ozone (O<sub>3</sub>), nitrogen monoxide (ON), nitrogen dioxide (NO<sub>2</sub>), dinitrogen monoxide (N<sub>2</sub>O), dinitrogen trioxide (N<sub>2</sub>O<sub>3</sub>), dinitrogen tetroxide (N<sub>2</sub>O<sub>4</sub>), dinitrogen pentoxide (N<sub>2</sub>O<sub>5</sub>), nitrogen trioxide, and lower siloxanes containing silicon atoms (Si), oxygen atoms (O) and hydrogen atoms (H) as constituent atoms such as disiloxane H<sub>3</sub>SiOSiH<sub>3</sub>, trisiloxane H<sub>3</sub>SiOSiH<sub>2</sub>OSiH<sub>3</sub>, and the like.

The starting materials which can effectively be used as the starting gas for introduction of nitrogen atoms (N) to be used in formation of the layer region (N) may include, for example, gaseous or gasifiable nitrogen compounds, nitrides and azides containing N, or N and H as constituent atoms for example, nitrogen (N<sub>2</sub>), ammonia (NH<sub>3</sub>), hydrazine (H<sub>2</sub>NNH<sub>2</sub>), hydrogen azide (HN<sub>3</sub>), ammonium azide (NH<sub>4</sub>N<sub>3</sub>) and so on. Alternatively, for the advantage of introducing halogen atoms (X) in addition to nitrogen atoms (N), there may be also employed nitrogen halide compounds such as nitrogen trifluoride (F<sub>3</sub>N), nitrogen tetrafluoride (F<sub>4</sub>N<sub>2</sub>) and the like.

For formation of the first layer (I) containing oxygen atoms and/or nitrogen atoms according to the sputtering method, a single crystalline or polycrystalline Si wafer and SiO<sub>2</sub> and/or Si<sub>3</sub>N<sub>4</sub> wafer or a wafer containing SiO<sub>2</sub> and/or Si<sub>3</sub>N<sub>4</sub> mixed therein may be employed and sputtering of these wafers may be conducted in various gas atmospheres.

For example, when Si wafer is employed as the target, a starting gas for introduction of oxygen atoms and/or nitrogen atoms optionally together with a starting gas for introduction of hydrogen atoms and/or halogen atoms, which may optionally be diluted with a diluting gas, may be introduced into a deposition chamber for sputtering to form gas plasma of these gases, in

which sputtering of the aforesaid Si wafer may be effected.

Alternatively, by use of separate targets of Si and SiO<sub>2</sub> and/or Si<sub>3</sub>N<sub>4</sub> or one sheet of a target containing SiO<sub>2</sub> and/or Si<sub>3</sub>N<sub>4</sub> mixed therein, sputtering may be effected in an atmosphere of a diluting gas as a gas for sputtering or in a gas atmosphere containing at least hydrogen atoms (H) or/and halogen atoms (X) as constituent atoms, whereby the first layer (I) having the layer region (ON) containing oxygen atoms and/or nitrogen atoms provided in the desired layer region can be formed.

As the starting gas for introduction of oxygen atoms and/or nitrogen atoms, there may be employed the starting gases shown as examples in the glow discharge method previously described also as effective gases in case of sputtering.

For incorporating a substance (C) for controlling conductivity such as the group III atoms or the group V atoms structurally into the layer region constituting the first layer (I), a starting material for introduction of the group III atoms or a starting material for introduction of the group V atoms may be introduced in a gaseous state into a deposition chamber together with the starting materials for formation of the first layer (I) during layer formation. As the starting material which can be used for introduction of the group III atoms, it is desirable to use those which are gaseous at room temperature under atmospheric pressure or can readily be gassified under layer forming conditions. Typical examples of such starting materials for introduction of the group III atoms, there may be included as the compounds for introduction of boron atoms, boron hydrides such as B<sub>2</sub>H<sub>6</sub>, B<sub>4</sub>H<sub>10</sub>, B<sub>5</sub>H<sub>9</sub>, B<sub>5</sub>H<sub>11</sub>, B<sub>6</sub>H<sub>10</sub>, B<sub>6</sub>H<sub>12</sub>, B<sub>6</sub>H<sub>14</sub>, etc. and boron halides such as BF<sub>3</sub>, BCl<sub>3</sub>, BBr<sub>3</sub>, etc. Otherwise, it is also possible to use AlCl<sub>3</sub>, GaCl<sub>3</sub>, Ga(CH<sub>3</sub>)<sub>3</sub>, InCl<sub>3</sub>, TiCl<sub>3</sub> and the like.

The starting materials which can effectively be used in the present invention for introduction of the group V atoms may include, for introduction of phosphorus atoms, phosphorus hydrides such as PH<sub>3</sub>, P<sub>2</sub>H<sub>4</sub>, etc., phosphorus halides such as PH<sub>4</sub>I, PF<sub>3</sub>, PF<sub>5</sub>, PCl<sub>3</sub>, PCl<sub>5</sub>, PBr<sub>3</sub>, PBr<sub>5</sub>, PI<sub>3</sub> and the like. Otherwise, it is also possible to utilize AsH<sub>3</sub>, AsF<sub>3</sub>, AsCl<sub>3</sub>, AsBr<sub>3</sub>, AsF<sub>5</sub>, SbH<sub>3</sub>, SbF<sub>3</sub>, SbF<sub>5</sub>, SbCl<sub>3</sub>, SbCl<sub>5</sub>, BiH<sub>3</sub>, BiCl<sub>3</sub>, BiBr<sub>3</sub> and the like effectively as the starting material for introduction of the group V atoms.

In the present invention, the content of the substance (C) for controlling conductivity in the first layer (I) may be suitably selected depending on the conductivity required for said first layer (I), or characteristics of other layers provided in direct contact with said first layer (I), the organic relationships such as relation with the characteristics of said other layers at the contacted interface, etc.

In the present invention, the content of the substance (C) for controlling conductivity contained in the first layer (I) should preferably be 0.01 to 5 × 10<sup>4</sup> atomic ppm, more preferably 0.5 to 1 × 10<sup>4</sup> atomic ppm, most preferably 1—5 × 10<sup>3</sup> atomic ppm.

In the present invention, the amount of hydrogen atoms (H) or the amount of halogen atoms (X) or the sum of the amounts of hydrogen atoms and halogen atoms (H+X) which may be contained in the first layer (I) should preferably be 1 to 40 atomic %, more preferably 5 to 30 atomic %.

For controlling the amount of hydrogen atoms (H) and/or halogen atoms (X) which may be contained in

the first layer (I), for example, the substrate temperature and/or the amount of the starting materials used for incorporation of hydrogen atoms (H) or halogen atoms (X) to be introduced into the deposition device system, discharging power, etc. may be controlled.

The first layer (I) of the present invention has a layer thickness which may suitably be determined as desired, depending on whether said first layer (I) acts primarily as the adhesion layer between the substrate and the second layer (II) or as the adhesion layer and the charge transporting layer. In the former case, it should desirably be 1000 Å to 50 μm, more preferably 2000 Å to 30 μm, most preferably 2000 Å to 10 μm. In the latter case, it should desirably be 1 to 100 μm, more preferably 1 to 80 μm, most preferably 2 to 50 μm.

In the photoconductive member of the present invention, a second layer (II) 104 is formed on the first layer (I) 103. The first layer (I) and the second layer (II) each comprise amorphous materials both having the common constituent atom of silicon atoms, and therefore chemical stability is sufficiently ensured at the laminated interface therebetween.

In the photoconductive member of the present invention, it is desirable that the germanium atoms contained in the second layer (II) should desirably take an ununiform distribution with respect to the layer thickness direction, but an uniform distribution with respect to the direction parallel to the surface of the substrate.

By forming the second layer (II) so as to have such a layer structure, a photoconductive member can be formed, which is excellent in photosensitivity to the light in the whole wavelength region from relatively shorter wavelengths to relatively longer wavelengths, including visible light region.

Also, as to the distribution state of germanium atoms in the second layer (II), it is possible to afford layer constitutions, for example, in which the distribution concentration C of germanium atoms in the thickness direction is distributed so as to be reduced from the boundary with the first layer (I) toward the boundary with the third layer (III), in which it is increased from the boundary with the first layer (I) toward the boundary with the third layer (III), or in which both of these characteristics are possessed.

FIGS. 2 through 13 show typical examples of distribution in the direction of layer thickness of germanium atoms contained in the second layer (II) of the photoconductive member in the present invention.

In FIGS. 2 through 13, the axis of abscissa indicates the distribution concentration C of germanium atoms and the axis of ordinate the layer thickness of the second layer (II), t<sub>B</sub> showing the position of the boundary between the first layer (I) and the second layer (II) and t<sub>T</sub> the position of the boundary between the second layer (II) and the third layer (III). That is, layer formation of the second layer (II) containing germanium proceeds from the t<sub>B</sub> side toward the t<sub>T</sub> side.

In FIG. 2, there is shown a first typical embodiment of the concentration depth profile of germanium atoms in the layer thickness direction contained in the second layer (II).

In the embodiment as shown in FIG. 2, from the interface position t<sub>B</sub> with the first layer (I), at which the second layer (II) containing germanium atoms is to be formed, to be position t<sub>1</sub>, germanium atoms are contained in the second layer (II) formed, while the distribution concentration C of the germanium atoms taking a constant value of C<sub>1</sub>, the concentration being gradu-

ally decreased from the concentration  $C_2$  continuously from the position  $t_1$  to interface position  $t_7$  of the third layer (III). At the interface position  $t_7$ , the concentration  $C$  of germanium atoms is made  $C_3$ .

In the embodiment shown in FIG. 3, the concentration  $C$  of germanium atoms contained is decreased gradually and continuously from the position  $t_B$  to the position  $t_7$  from the concentration  $C_4$  until it becomes the concentration  $C_5$  at the position  $t_7$ .

In case of FIG. 4, the concentration  $C$  of germanium atoms is made constant as  $C_6$  from the position  $t_B$  to the position  $t_2$ , gradually decreased continuously from the position  $t_2$  to the position  $t_7$  and the concentration  $C$  is made substantially zero at the position  $t_7$  (substantially zero herein means the content less than the detectable limit).

In case of FIG. 5, the distribution concentration  $C$  of germanium atoms are decreased gradually and continuously from the position  $t_B$  to the position  $t_7$  from the concentration  $C_8$ , until it is made substantially zero at the position  $t_7$ .

In the embodiment shown in FIG. 6, the distribution concentration  $C$  of germanium atoms is constantly  $C_9$  between the position  $t_B$  and the position  $t_3$ , and it is made  $C_{10}$  at the position  $t_7$ . Between the position  $t_3$  and the position  $t_7$ , the distribution concentration  $C$  is decreased as a first order function from the position  $t_3$  to the position  $t_7$ .

In the embodiment shown in FIG. 7, there is formed a concentration depth profile such that the distribution concentration  $C$  takes a constant value of  $C_{11}$  from the position  $t_B$  to the position  $t_4$ , and is decreased as a first order function from the concentration  $C_{12}$  concentration  $C_{13}$  from the position  $t_4$  to the position  $t_7$ .

In the embodiment shown in FIG. 8, the distribution concentration  $C$  of germanium atoms is decreased linearly from the concentration  $C_{14}$  to substantially zero from the position  $t_B$  to the position  $t_7$ .

In FIG. 9, there is shown an embodiment, where the concentration  $C$  of germanium atoms is decreased linearly from the concentration  $C_{15}$  to  $C_{16}$  from the position  $t_B$  to  $t_7$  and made constantly at the concentration  $C_{16}$  between the position  $t_5$  and  $t_7$ .

In the embodiment shown in FIG. 10, the concentration  $C$  of germanium atoms is at the concentration  $C_{17}$  at the position  $t_B$ , which concentration  $C_{17}$  is initially decreased gradually and abruptly near the position  $t_6$  to the position  $t_6$ , until it is made the concentration  $C_{18}$  at the position  $t_6$ .

Between the position  $t_6$  and the position  $t_7$ , the concentration is initially decreased abruptly and thereafter gradually, until it is made the concentration  $C_{19}$  at the position  $t_7$ . Between the position  $t_7$  and the position  $t_8$ , the concentration is decreased very gradually to the concentration  $C_{20}$  at the position  $t_8$ . Between the position  $t_8$  and the position  $t_7$ , the concentration is decreased along the curve having a shape as shown in the Figure from the concentration  $C_{20}$  to substantially zero.

In the embodiment shown in FIG. 11, the germanium concentration is constantly  $C_{22}$  from the position  $t_B$  to the position  $t_9$ , and the germanium concentration  $C$  is made constantly  $C_{21}$  from the position  $t_9$  to the position  $t_B$ .

In the embodiment shown in FIG. 12, the germanium concentration is substantially zero at the position  $t_7$ , and is increased along the curve as shown in the Figure so that it may become  $C_{23}$  at the position  $t_7$ .

In FIG. 13, the germanium concentration is substantially zero at the position  $t_B$ , and the germanium concentration is increased along the curve as shown in the figure from the position  $t_B$  to the concentration  $C_{24}$  at the position  $t_{10}$ , the germanium concentration being constantly  $C_{24}$  from the position  $t_{10}$  to the position  $t_7$ .

In the germanium concentration depth profiles shown in FIGS. 2 through 13, the germanium concentration is enriched in the vicinity of the boundary interface of the first layer (I) in FIGS. 2 through 10, while the germanium concentration enriched in the vicinity of the boundary interface of the third layer (III) in FIGS. 1 through 13. It is also possible to use a combination of three germanium concentration depth profiles.

As described above about some typical examples of depth profiles of germanium atoms contained in the second layer (II) in the direction of the layer thickness by referring to FIGS. 2 through 13, in the present invention, a portion with higher distribution concentration  $C$  of germanium atoms lies in the vicinity of the boundary interface of the first layer (I) and/or of the third layer (III), while there is provided in the second layer (II) a distribution state of germanium atoms having a portion with considerably lower concentration as compared with the vicinity of the boundary interface of the first layer (I) and of the third layer (III).

The second layer (II) constituting the light-receiving layer of the photoconductive member in the present invention is desired to have a localized region (A) containing germanium atoms preferably at a relatively higher concentration in the vicinity of the boundary interface of the first layer (I) or of the third layer (III) as described above.

In the present invention, the localized region (A), as explained in terms of the symbols shown in FIG. 2 through FIG. 13, may be desirably provided within  $5\mu$  from the interface position  $t_B$  or  $t_7$ .

In the present invention, the above localized region (A) may be made to occupy the whole layer region ( $L_7$ ) from the interface position  $t_B$  or  $t_7$  to the thickness of  $5\mu$  or alternatively a part of the layer region ( $L_7$ ).

It may suitably be determined depending on the characteristics required for the light-receiving layer to be formed, whether the localized region (A) is made a part or whole of the layer region ( $L_7$ ).

The localized region (A) may preferably be formed according to such a layer formation that the maximum value  $C_{max}$  of the concentration  $C$  of germanium atoms in a distribution in the layer thickness direction may preferably be 1000 atomic ppm or more, more preferably 5000 atomic ppm or more, most preferably  $1\times 10^4$  atomic ppm or more.

That is, according to the present invention, the second layer (II) containing germanium atoms is formed so that the maximum value  $C_{max}$  of the distribution concentration may exist within a layer thickness of  $5\mu$  from the first layer (I) side or from the free surface of the second layer (II) (the layer region within thickness of  $5\mu$  from  $t_B$ ).

In the present invention, the content of germanium atoms in the second layer (II) containing germanium atoms, which may suitably be determined as desired so as to achieve effectively the objects of the present invention, may preferably be  $1$  to  $9.5\times 10^5$  atomic ppm, more preferably 100 to  $8\times 10^5$  atomic ppm, most preferably 500 to  $7\times 10^5$  atomic ppm.

In the photoconductive member of the present invention, for the purpose of effecting higher sensitization

and higher dark resistance, or further improving adhesion between the first layer (I) and the second layer (II) of between the second layer (II) and the third layer (III), or adhesion of the first layer (I), the second layer (II) and the third layer (III), the second layer (II) should desirably contain oxygen atoms and/or nitrogen atoms.

The oxygen atoms and/or nitrogen atoms contained in the second layer (II) may be contained either evenly throughout the whole region or only in a part of the region.

The distribution C(ON) of oxygen atoms and/or nitrogen atoms may be either uniform or ununiform in the layer thickness direction of the second layer (II).

In the present invention, the layer region (ON) containing oxygen atoms and/or nitrogen atoms provided on the second layer (II) is provided so as to occupy the whole layer region of the second layer (II) when it is intended to improve photosensitivity and dark resistance, while it is provided so as to occupy the end portion layer region of the first layer (I) and/or the third layer (III) when it is intended to strengthen adhesion with the first layer (I) and/or the third layer (III).

The content of oxygen atoms and/or nitrogen atoms to be contained in the layer region (ON) provided in such a second layer (II) can be selected suitably depending on the characteristics required for the layer region (ON) itself so as to accomplish the objects as mentioned above, the characteristics required at the contacted interface with the first layer (I) or the third layer (III) or the organic relationships with the characteristics of the first layer (I) or the third layer (III).

The content of oxygen atoms and/or nitrogen atoms in the layer region (ON), which may be determined suitably as desired depending on the characteristics of the photoconductive member to be formed, may be preferably 0.001 to 50 atomic %, more preferably 0.002 to 40 atomic %, most preferably 0.003 to 30 atomic %.

In the photoconductive member of the present invention, when the first layer (I) has a thin thickness, a layer region (PN) containing a substance (C) for controlling conductivity can be provided in the second layer (II) containing germanium atoms locally on the first layer (I) side, whereby said layer region can function as the so-called charge injection impeding layer.

That is, by making the content of the substance (C) for controlling conductivity in the layer region (PN) preferably 30 atomic ppm or more, more preferably 50 atomic ppm or more, most preferably 100 atomic ppm or more, for example, in the case when said substance (C) to be incorporated is a p-type impurity as mentioned above, migration of electrons injected from the substrate side into the light-receiving layer can be effectively inhibited when the free surface of the light-receiving layer is subjected to the charging treatment to  $\ominus$ polarity. On the other hand, when the substance to be incorporated is a n-type impurity, migration of positive holes injected from the substrate side into the light-receiving layer can be effectively inhibited when the free surface of the light-receiving layer is subjected to the charging treatment to  $\oplus$ polarity.

In the case as mentioned above, the layer region (ZII) at the portion of the second layer (II) excluding the above layer region (PN) under the basic constitution of the present invention as described above may contain a substance (C) for controlling conductivity of the other polarity, or a substance (C) for controlling conductivity characteristics of the same polarity may be contained

therein in an amount by far smaller than that practically contained in the layer region (PN).

In such a case, the content of the substance (C) for controlling conductivity contained in the above layer region (ZII) can be determined adequately as desired depending on the polarity or the content of the substance contained in the layer region (PN), but it is preferably 0.001 to 1000 atomic ppm, more preferably 0.05 to 500 atomic ppm, most preferably 0.1 to 200 atomic ppm.

In the present invention, when the same kind of a substance (C) for controlling conductivity is contained in the layer region (PN) and the layer region (ZII), the content in the layer region (ZII) should preferably be 30 atomic ppm or less. Being different from the cases as mentioned above, in the present invention, it is also possible to provide in the second layer (II) a layer region containing a substance (C) for controlling conductivity having one polarity and a layer region containing a substance (C) for controlling conductivity having the other polarity in direct contact with each other, thus providing a so-called depletion layer at said contact region. In short, for example, a layer containing the aforesaid p-type impurity and a layer region containing the aforesaid n-type impurity are provided in the light-receiving layer in direct contact with each other to form the so-called p-n junction, whereby a depletion layer can be provided.

In the present invention, illustrative of halogen atoms (X), which may optionally be incorporated in the second layer (II) are fluorine, chlorine, bromine and iodine, particularly preferably fluorine and chlorine.

In the present invention, formation of the second layer (II) constituted of a-SiGe(H,X) may be conducted according to the vacuum deposition method utilizing discharging phenomenon, such as glow discharge method, sputtering method or ion-plating method.

For example, for formation of the second layer (II) constituted of a-SiGe(H,X) according to the glow discharge method, the basic procedure comprises introducing a starting gas for Si supply capable of supplying silicon atoms (Si), a starting gas for Ge optionally together with a starting gas for introduction of hydrogen atoms (H) and/or halogen atoms (X) into a deposition chamber which can be internally brought to a state of reduced pressure, and exciting glow discharge in said deposition chamber, thereby effecting layer formation on the surface of a substrate, on which the first layer (I) has been formed, and placed at a predetermined position, while controlling the concentration depth profile of germanium atoms according to a desired change rate curve to form the second layer (II) constituted of a-SiGe(H,X).

Alternatively, for formation according to the sputtering method, when carrying out sputtering by use of a target constituted of Si or two sheets of targets of said target and a target constituted of Ge, or a target of a mixture of Si and Ge in an atmosphere of an inert gas such as Ar, He, etc. or a gas mixture based on these gases, a starting gas for Ge supply optionally together with, if desired, a gas for introduction of hydrogen atoms (H) and/or halogen atoms (X) may be introduced into a deposition chamber for sputtering, thereby forming a plasma atmosphere and effecting the sputtering of the above-mentioned target, while controlling the flow rate of the starting gas according to a desired change rate curve.

In the case of the ion-plating method, for example, a vaporizing source such as a polycrystalline silicon or a single crystalline silicon and a polycrystalline germanium or a single crystalline germanium may be placed as vaporizing source in an evaporating boat, and the vaporizing source is heated by the resistance heating method or the electron beam method (EB method) to be vaporized, and the flying vaporized product is permitted to pass through a desired gas plasma atmosphere, otherwise following the same procedure as in the case of sputtering.

In the present invention, as the effective starting materials for the starting gases to be employed for formation of the second layer (II), the following compounds may be included.

First, the starting gas for supplying Si to be used in the present invention may include gaseous or gasifiable hydrogenated silicones (silanes) such as  $\text{SiH}_4$ ,  $\text{Si}_2\text{H}_6$ ,  $\text{Si}_3\text{H}_8$ ,  $\text{Si}_4\text{H}_{10}$  and others as effective materials. In particular,  $\text{SiH}_4$  and  $\text{Si}_2\text{H}_6$  are preferred with respect to easy handling during layer formation and efficiency for supplying Si. As the substances which can be starting gases for Ge supply, there may be effectively employed gaseous or gasifiable hydrogenated germanium such as  $\text{GeH}_4$ ,  $\text{Ge}_2\text{H}_6$ ,  $\text{Ge}_3\text{H}_8$ ,  $\text{Ge}_4\text{H}_{10}$ ,  $\text{Ge}_5\text{H}_{12}$ ,  $\text{Ge}_6\text{H}_{12}$ ,  $\text{Ge}_7\text{H}_{16}$ ,  $\text{Ge}_8\text{H}_{18}$ ,  $\text{Ge}_9\text{H}_{20}$ , etc. In particular,  $\text{GeH}_4$ ,  $\text{Ge}_2\text{H}_6$  and  $\text{Ge}_3\text{H}_8$  are preferred with respect to easy handling during layer formation and efficiency for supplying Ge.

Effective starting gases for introduction of halogen atoms (X) to be used for formation of the second layer (II) in the present invention may include a large number of halogen compounds, as exemplified preferably be halogen gases, halides, interhalogen compounds, or gaseous or gasifiable halogen compounds such as silane derivatives substituted with halogens. Further, there may also be included gaseous or gasifiable silicon compounds containing halogen atoms constituted of silicon atoms and halogen atoms as constituent elements as effective ones in the present invention.

Typical examples of halogen compounds preferably used for formation of the second layer (II) in the present invention may include halogen gases such as fluorine, chlorine, bromine or iodine, interhalogen compounds such as  $\text{ClF}$ ,  $\text{ClF}_3$ ,  $\text{BrF}$ ,  $\text{BrF}_3$ ,  $\text{BrF}_5$ ,  $\text{IF}_3$ ,  $\text{IF}_7$ ,  $\text{ICl}$ ,  $\text{IBr}$ , etc.

As the silicon compounds containing halogen atoms (X), namely so called silane derivatives substituted with halogens, there may preferably be employed silicon halides such as  $\text{SiF}_4$ ,  $\text{Si}_2\text{H}_6$ ,  $\text{SiCl}_4$ ,  $\text{SiBr}_4$  and the like.

When the second layer (II) in the photoconductive member of the present invention is formed according to the glow discharge method by employing such a silicon compound containing halogen atoms (X), it is possible to form the second layer (II) constituted of a-SiGe(H,X) containing halogen atoms on a substrate, having the first layer (I) formed on its surface, without use of a hydrogenated silicon gas as the starting gas capable of supplying Si together with the starting gas for Ge supply.

In the case of forming the second layer (II) containing halogen atoms (X) according to the glow discharge method, the basic procedure comprises introducing, for example, a silicon halide as the starting gas for Si supply, a hydrogenated germanium as the starting gas for Ge supply and a gas such as Ar,  $\text{H}_2$ , He, etc. at a predetermined mixing ratio into the deposition chamber for formation of the second layer (II) and exciting glow discharge to form a plasma atmosphere of these gases,

whereby the second layer (II) can be formed on a substrate having the first layer (I) formed on its surface. In order to control the ratio of hydrogen atoms incorporated more easily, hydrogen gas or a gas of a silicon compound containing hydrogen atoms may also be mixed with these gases in a desired amount to form the second layer (II). Also, each gas is not restricted to a single species, but multiple species may be used at any desired ratio.

In either case of the sputtering method and the ion-plating method, introduction of halogen atoms (X) into the layer formed may be performed by introducing the gas of the above halogen compound or the above silicon compound containing halogen atoms into a deposition and forming a plasma atmosphere of said gas.

On the other hand, for introduction of hydrogen atoms, a starting gas for introduction of hydrogen atoms, for example,  $\text{H}_2$  or gases such as silanes and/or hydrogenated germanium as mentioned above, may be introduced into a deposition chamber for sputtering, followed by formation of the plasma atmosphere of said gases.

In the present invention, as the starting gas for introduction of halogen atoms during formation of the second layer (II), the halides or halogen-containing silicon compounds as mentioned above can effectively be used. Otherwise, it is also possible to use effectively as the starting material for formation of the second layer (II) gaseous or gasifiable substances, including halides containing hydrogen atom as one of the constituents, e.g. hydrogen halide such as  $\text{HF}$ ,  $\text{HCl}$ ,  $\text{HBr}$ ,  $\text{HI}$ , etc.; halogen-substituted hydrogenated silicon such as  $\text{SiH}_2\text{F}_2$ ,  $\text{SiH}_2\text{I}_2$ ,  $\text{SiH}_2\text{Cl}_2$ ,  $\text{SiHCl}_3$ ,  $\text{SiH}_2\text{Br}_2$ ,  $\text{SiHBr}_3$ , etc.; hydrogenated germanium halides such as  $\text{GeHF}_3$ ,  $\text{GeH}_2\text{F}_2$ ,  $\text{GeH}_3\text{F}$ ,  $\text{GeHCl}_3$ ,  $\text{GeH}_2\text{Cl}_2$ ,  $\text{GeH}_3\text{Cl}$ ,  $\text{GeHBr}_3$ ,  $\text{GeH}_2\text{Br}_2$ ,  $\text{GeH}_3\text{Br}$ ,  $\text{GeHI}_3$ ,  $\text{GeH}_2\text{I}_2$ ,  $\text{GeH}_3\text{I}$ , etc.; germanium halides such as  $\text{GeF}_4$ ,  $\text{GeCl}_4$ ,  $\text{GeBr}_4$ ,  $\text{GeI}_4$ ,  $\text{GeF}_2$ ,  $\text{GeCl}_2$ ,  $\text{GeBr}_2$ ,  $\text{GeI}_2$ , etc.

Among these substances, halides containing hydrogen atoms can preferably be used as the starting material for introduction of halogens, because hydrogen atoms, which are very effective for controlling electrical or photoelectric characteristics, can be introduced into the layer simultaneously with introduction of halogen atoms during formation of the second layer (II).

For introducing hydrogen atoms structurally into the second layer (II), other than those as mentioned above,  $\text{H}_2$  or a hydrogenated silicon such as  $\text{SiH}_4$ ,  $\text{Si}_2\text{H}_6$ ,  $\text{Si}_3\text{H}_8$ ,  $\text{Si}_4\text{H}_{10}$ , etc. together with germanium or a germanium compound for supplying Ge, or a hydrogenated germanium such as  $\text{GeH}_4$ ,  $\text{Ge}_2\text{H}_6$ ,  $\text{Ge}_3\text{H}_8$ ,  $\text{Ge}_4\text{H}_{10}$ ,  $\text{Ge}_5\text{H}_{12}$ ,  $\text{Ge}_6\text{H}_{14}$ ,  $\text{Ge}_7\text{H}_{16}$ ,  $\text{Ge}_8\text{H}_{18}$ ,  $\text{Ge}_9\text{H}_{20}$ , etc. together with silicon or a silicon compound for supplying Si can be permitted to co-exist in a deposition chamber, followed by excitation of discharging.

According to a preferred embodiment of the present invention, the amount of hydrogen atoms (H) or the amount of halogen atoms (X) or the sum of the amounts of hydrogen atoms and halogen atoms (H+X) to be contained in the second layer (II) constituting the light-receiving layer to be formed should preferably be 0.01 to 40 atomic %, more preferably 0.05 to 30 atomic %, most preferably 0.1 to 25 atomic %.

For controlling the amount of hydrogen atoms (H) and/or halogen atoms (X) to be contained in the second layer (II), for example, the substrate temperature and/or the amount of the starting materials used for incorporation of hydrogen atoms (H) or halogen atoms (X)

to be introduced into the deposition device system, discharging power, etc. may be controlled.

For incorporating a substance (C) for controlling conductivity such as the group III atoms or the group V atoms structurally into the second layer (II), a starting material for introduction of the group III atoms or a starting material for introduction of the group V atoms may be introduced under gaseous state into a deposition chamber together with other starting materials for formation of the second layer (II) during layer formation, similarly to that described about formation of the first layer (I).

The second layer (II) in the photoconductive member of the present invention may have a thickness, which may be determined in view of the absorption coefficient of the second layer (II) relative to the photo-carrier excitation light source, when the second layer (II) is used primarily for photocarrier generating layer, and it may preferably be made 1000 Å to 50 μm, more preferably 1000 Å to 30 μm, most preferably 1000 Å to 20 μm.

On the other hand, when the second layer (II) is used primarily as the layer for generation and transportation of photocarriers, the thickness may be determined suitably as desired so that the photocarriers may be transported with good efficiency, and may preferably be made 1 to 100 μm, more preferably 1 to 80 μm, most preferably 2 to 50 μm.

In the present invention, when a layer region (ON) containing at least one of oxygen atoms and nitrogen atoms is provided in the second layer (II), a starting material for introduction of oxygen atoms and/or nitrogen atoms may be used in combination while controlling its amount during formation of the layer by use of the above starting materials thereby incorporating oxygen atoms and/or nitrogen atoms in the layer formed.

When the glow discharge method is applied for formation of the layer region (ON), the starting materials for introduction of oxygen atoms and/or nitrogen atoms are further added to those selected as desired from among the starting materials for formation of the second layer (II). As such starting materials for introduction of oxygen atoms and/or nitrogen atoms, most of gaseous or gasified gasifiable substances having oxygen atoms or and nitrogen atoms as constituent atoms may be employed.

As the starting materials effectively used for supplying oxygen atoms (O) for formation of the layer region (ON), there may be employed a starting gas containing (O) as constituent atoms or a starting gas containing (O) and (H) as constituent atoms, for example, oxygen (O<sub>2</sub>), ozone (O<sub>3</sub>), nitrogen monoxide (NO), nitrogen dioxide (NO<sub>2</sub>), dinitrogen monoxide (N<sub>2</sub>O), dinitrogen trioxide (N<sub>2</sub>O<sub>3</sub>), dinitrogen tetroxide (N<sub>2</sub>O<sub>4</sub>), dinitrogen pentoxide (N<sub>2</sub>O<sub>5</sub>), nitrogen trioxide, and lower siloxanes containing silicon atoms (Si), oxygen atoms (O) and hydrogen atoms (H) as constituent atoms such as disiloxane (H<sub>3</sub>SiOSiH<sub>3</sub>), trisiloxane (H<sub>3</sub>SiOSiH<sub>2</sub>OSiH<sub>3</sub>), and the like.

The starting materials which can effectively be used as the starting gas for introduction of nitrogen atoms (N) to be used in formation of the layer region (ON) may include, for example, gaseous or gasifiable nitrogen compounds, nitrides and azides containing N, or N and H as constituent atoms, for example, nitrogen (N<sub>2</sub>), ammonia (NH<sub>3</sub>), hydrazine (H<sub>2</sub>NNH<sub>2</sub>), hydrazine azide (HN<sub>3</sub>), ammonium azide (NH<sub>4</sub>N<sub>3</sub>) and so on. Alternatively, for the advantage of introducing halogen atoms

(X) in addition to nitrogen atoms (N), there may be also employed nitrogen halide compounds such as nitrogen trifluoride (F<sub>3</sub>N), nitrogen tetrafluoride (F<sub>4</sub>N<sub>2</sub>) and the like.

In the present invention, when providing layer region (ON) containing oxygen atoms and/or nitrogen atoms during formation of the first layer (I) and the second layer (II) in at least one of these layers, formation of the layer region (ON) having a desired depth profile in the direction of layer thickness formed by varying the distribution concentration C(ON) of oxygen atoms and/or nitrogen atoms contained in said layer region (ON) may be conducted in case of glow discharge by introducing a starting gas for introduction of oxygen atoms and/or nitrogen atoms of which the distribution concentration C(ON) is to be varied into a deposition chamber, while varying suitably its gas flow rate according to a desired change rate curve.

In case when sputtering is employed, for example, when a target containing Si, SiO<sub>2</sub> and/or Si<sub>3</sub>N<sub>4</sub> mixed therein is used as the target for sputtering, the mixing ratio of Si to SiO<sub>2</sub> and/or Si<sub>3</sub>N<sub>4</sub> may be previously varied in the layer thickness direction of the target, whereby a desired depth profile of oxygen atoms and/or nitrogen atoms in the layer thickness direction can be obtained.

The third layer (III) 105 to be formed on the second layer (II) 104 in the photoconductive member of the present invention has a free surface and is provided primarily for the purpose of accomplishing the objects of the present invention with respect to humidity resistance, continuous repeated use characteristics, dielectric strength, environmental use characteristics and durability. Since each of the second layer (II) and the third layer (III) comprises an amorphous material having common constituent atoms of silicon atoms, chemical stability is sufficiently ensured at the laminated interface.

The third layer (III) in the present invention is constituted of an amorphous material containing silicon atoms (Si) and carbon atoms (C), optionally together with hydrogen atoms (H) and/or halogen atoms (X) (hereinafter referred to as "a-(Si<sub>x</sub>C<sub>1-x</sub>)<sub>y</sub>(H,X)<sub>1-y</sub>", where 0 < x, y < 1).

Formation of the third layer (III) constituted of a-(Si<sub>x</sub>C<sub>1-x</sub>)<sub>y</sub>(H,X)<sub>1-y</sub> may be performed according to the glow discharge method, the sputtering method, the ion implantation method, the ion plating method, the electron beam method, etc. These preparation methods may be suitably selected depending on various factors such as the preparation conditions, the degree of the load for capital investment for installations, the production scale, the desirable characteristics required for the photoconductive member to be prepared, etc. For the advantages of relatively easy control of the preparation conditions for preparing photoconductive members having desired characteristics and easy introduction of carbon atoms and/or halogen atoms together with silicon atoms, into the third layer (III) to be prepared, there may preferably be employed the glow discharge method or the sputtering method. Further, the third layer (III) may be formed by using the glow discharge method and the sputtering method in combination in the same device system.

For formation of the third layer (III) according to the glow discharge method, starting gases for formation of a-(Si<sub>x</sub>C<sub>1-x</sub>)<sub>y</sub>(H,X)<sub>1-y</sub>, optionally mixed at a predetermined mixing ratio with diluting gas, may be introduced

into a deposition chamber for vacuum deposition in which a substrate having the second layer (II) formed thereon is placed, and the gas introduced is made into a gas plasma by excitation of glow discharging, thereby depositing a-( $\text{Si}_x\text{C}_{1-x}$ )<sub>y</sub>(H,X)<sub>1-y</sub> on the second layer (II) which has already been formed on the aforesaid support.

As the starting gases for formation of a-( $\text{Si}_x\text{C}_{1-x}$ )<sub>y</sub>(H,X)<sub>1-y</sub> to be used in the present invention, it is possible to use most of gaseous substances or gasified gasifiable substances containing at least one of silicon atoms (Si), carbon atoms (C), hydrogen atoms (H) and halogen atoms (X) as constituent atoms.

In case when a starting gas having Si as constituent atoms as one of Si, C, H and X is employed, there may be employed, for example, a mixture of a starting gas containing Si as constituent atom with a starting gas containing C as constituent atom, and optionally with a starting gas containing H and/or X as a constituent atom at a desired mixing ratio, or alternatively a mixture of a starting gas containing Si as constituent atoms with a gas containing three atoms of Si, C and H or of Si, C and X as constituent atoms at a desired mixing ratio.

Alternatively, it is also possible to use a mixture of a starting gas containing Si and H as constituent atoms with a starting gas containing C as constituent atom or a mixture of a starting gas containing C as constituent atom.

In the present invention, preferable halogen atoms (X) to be contained in the third amorphous layer (III) are F, Cl, Br and I. Particularly, F and Cl are preferred.

In the present invention, the starting gases effectively used for formation of the third layer (III) may include hydrogenated silicon gases containing Si and H as constituent atoms such as silanes (e.g.  $\text{SiH}_4$ ,  $\text{Si}_2\text{H}_6$ ,  $\text{Si}_3\text{H}_8$ ,  $\text{Si}_4\text{H}_{10}$ , etc.), compounds containing C and H as constituent atoms such as saturated hydrocarbons of 1 to 5 carbon atoms, ethylenic hydrocarbons having 2 to 4 carbon atoms and acetylenic hydrocarbons having 2 to 4 carbon atoms; simple substances of halogen; hydrogen halides; interhalogen compounds; halogenated silicon; halo-substituted hydrogenated silicon; etc.

More specifically, there may be included, as saturated hydrocarbons, methane( $\text{CH}_4$ ), ethane ( $\text{C}_2\text{H}_6$ ), propane ( $\text{C}_3\text{H}_8$ ), n-butane ( $\text{n-C}_4\text{H}_{10}$ ), pentane ( $\text{C}_5\text{H}_{12}$ ); as ethylenic hydrocarbons, ethylene ( $\text{C}_2\text{H}_4$ ), propylene ( $\text{C}_3\text{H}_6$ ), butene-1 ( $\text{C}_4\text{H}_8$ ), butene-2 ( $\text{C}_4\text{H}_8$ ), isobutylene ( $\text{C}_4\text{H}_8$ ), pentene ( $\text{C}_5\text{H}_{10}$ ); as acetylenic hydrocarbons, acetylene ( $\text{C}_2\text{H}_2$ ), methyl acetylene ( $\text{C}_3\text{H}_4$ ), butyne ( $\text{C}_4\text{H}_6$ ); halogen gases such as fluorine, chlorine, bromine and iodine; hydrogen halides such as HF, HI, HCl and HBr; interhalogen compounds such as CIF, CIF<sub>3</sub>, BrF<sub>5</sub>, BrF, BrF<sub>3</sub>, BrF<sub>5</sub>, IF<sub>3</sub>, IF<sub>7</sub>, ICl, IBr; halogenated silicon such as SiF<sub>4</sub>, Si<sub>2</sub>F<sub>6</sub>, SiCl<sub>4</sub>, SiCl<sub>3</sub>Br, SiCl<sub>2</sub>Br<sub>2</sub>, SiClBr<sub>3</sub>, SiCl<sub>3</sub>I, SiBr<sub>4</sub>, etc., halo-substituted hydrogenated silicon, including SiH<sub>2</sub>F<sub>2</sub>, SiH<sub>2</sub>Cl<sub>2</sub>, SiHCl<sub>3</sub>, SiH<sub>3</sub>Cl, SiH<sub>3</sub>Br, SiH<sub>2</sub>Br<sub>2</sub>, SiHBr<sub>3</sub>, etc.

In addition to these materials, there may also be employed halo-substituted paraffinic hydrocarbons such as CF<sub>4</sub>, CCl<sub>4</sub>, CBr<sub>4</sub>, CHF<sub>3</sub>, CH<sub>2</sub>F<sub>2</sub>, CH<sub>3</sub>F, CH<sub>3</sub>Cl, CH<sub>3</sub>Br, CH<sub>3</sub>I, C<sub>2</sub>H<sub>5</sub>Cl and the like, fluorinated sulfur compounds such as SF<sub>4</sub>, SF<sub>6</sub> and the like, silanes such as Si(CH<sub>3</sub>)<sub>4</sub>, Si(C<sub>2</sub>H<sub>5</sub>)<sub>4</sub> and the like; halo-containing alkyl silanes such as SiCl(CH<sub>3</sub>)<sub>3</sub>, SiCl<sub>2</sub>(CH<sub>3</sub>)<sub>2</sub>, SiCl<sub>3</sub>CH<sub>3</sub> and the like, as effective materials.

These substances for forming the third layer (III) may be chosen as desired and used during formulation of the third layer (III) so that silicon atoms, carbon

atoms and, if desired, halogen atoms and/or hydrogen atoms may be contained in the third layer (III) formed at a predetermined composition ratio.

For example, Si(CH<sub>3</sub>)<sub>4</sub> as the material capable of incorporating easily silicon atoms, carbon atoms and hydrogen atoms and forming a layer having desired characteristics and SiHCl<sub>3</sub>, SiCl<sub>4</sub>, SiH<sub>2</sub>Cl<sub>2</sub> or SiH<sub>3</sub>Cl as the starting material for incorporating halogen atoms may be mixed at a predetermined mixing ratio and introduced in a gaseous state into the device for formation of the third layer (III), followed by excitation of glow discharge, whereby there can be formed a third layer (III) comprising a-( $\text{Si}_x\text{C}_{1-x}$ )<sub>y</sub>(H,X)<sub>1-y</sub>.

For formation of the third layer (III) according to the sputtering method, a single crystalline or polycrystalline Si wafer and/or C wafer or a wafer containing Si and C mixed therein is used as target and subjected to sputtering in an atmosphere of various gases containing, if desired, halogen atoms and/or hydrogen atoms as constituent elements.

For example, when Si wafer is used as target, starting gases for introducing C, H and/or X, which may be diluted with a diluting gas, if desired, is introduced into a deposition chamber for sputtering to form a gas plasma therein and effect sputtering of said Si wafer.

Alternatively, Si and C as separate targets or one sheet target of a mixture of Si and C can be used and sputtering is effected in a gas atmosphere containing, if necessary, hydrogen atoms or halogen atoms. As the starting gas for introduction of C, H and X, there may be employed those for formation of the third layer (III) as mentioned in the glow discharge as described above as effective gases also in case of sputtering.

In the present invention, as the diluting gas to be used in forming the third layer (III) by the glow discharge method or the sputtering method, there may be preferably employed so-called rare gases such as He, Ne, Ar and the like.

The third layer (III) in the present invention should be carefully formed so that the required characteristics may be given exactly as desired.

That is, a substance containing as constituent atoms Si, C and, if necessary, H and/or X may take various forms from crystalline to amorphous, electrical properties from conductive through semi-conductive to insulating and photoconductive properties from photoconductive to non-photoconductive depending on the preparation conditions. Therefore, in the present invention, the preparation conditions are carefully selected as desired so that there may be formed a-( $\text{Si}_x\text{C}_{1-x}$ )<sub>y</sub>(H,X)<sub>1-y</sub> having desired characteristics depending on the purpose. For example, when the third layer (III) is to be provided primarily for the purpose of improvement of dielectric strength, a-( $\text{Si}_x\text{C}_{1-x}$ )<sub>y</sub>(H,X)<sub>1-y</sub> is prepared as an amorphous material having marked electric insulating behaviors under the use conditions.

Alternatively, when the primary purpose for provision of the third layer (III) is improvement of continuous repeated use characteristics or environmental characteristics during use, the degree of the above electric insulating property may be alleviated to some extent and a-( $\text{Si}_x\text{C}_{1-x}$ )<sub>y</sub>(H,X)<sub>1-y</sub> may be prepared as an amorphous material having sensitivity to some extent to the light irradiated.

In forming the third layer (III) comprising a-( $\text{Si}_x\text{C}_{1-x}$ )<sub>y</sub>(H,X)<sub>1-y</sub> on the surface of the second layer (II), the substrate temperature during layer formation is an important factor having influences on the structure

and the characteristics of the layer to be formed, and it is desired in the present invention to control severely the substrate temperature during layer formation so that  $a\text{-}(\text{Si}_x\text{C}_{1-x})_y(\text{H},\text{X})_{1-y}$  having intended characteristics may be prepared as desired.

As the substrate temperature in forming the third layer (III) for accomplishing effectively the objects in the present invention, there may be selected suitably the optimum temperature range in conformity with the method for forming the third layer (III) in carrying out formation of the third layer (III), preferably be 20° to 400° C., more preferably 50° to 350° C., most preferably 100° to 300° C. For formation of the third layer (III), the glow discharge method or the sputtering method may be advantageously adopted, because severe control of 15 the composition ratio of atoms constituting the layer or control of layer thickness can be conducted with relative ease as compared with other methods. In case when the third layer (III) is to be formed according to these 20 layer forming methods, the discharging power during layer formation is one of the important factors influencing the characteristics of  $a\text{-}(\text{Si}_x\text{C}_{1-x})_y(\text{H},\text{X})_{1-y}$  to be prepared, similarly as the aforesaid substrate temperature.

The discharging power condition for preparing effectively  $a\text{-}(\text{Si}_x\text{C}_{1-x})_y(\text{H},\text{X})_{1-y}$  having characteristics for accomplishing the objects of the present invention with good productivity may preferably be 10 to 300 W, more preferably 20 to 250 W, most preferably 50 to 200 W.

The gas pressure in a deposition chamber may preferably be 0.01 to 1 Torr, more preferably 0.1 to 0.5 Torr.

In the present invention, the above numerical ranges may be mentioned as preferable numerical ranges for the substrate temperature, discharging power, etc., for preparation of the third layer (III). However, these 35 factors for layer formation should not be determined separately independently of each other, but it is desirable that the optimum values of respective layer forming factors should be determined based on mutual organic relationships so that a third layer (III) comprising  $a\text{-}(\text{Si}_x\text{C}_{1-x})_y(\text{H},\text{X})_{1-y}$  having desired characteristics may be formed.

The content of carbon atoms in the third layer (III) in the photoconductive member of the present invention is one of the important factors for obtaining the desired 45 characteristics to accomplish the objects of the present invention, similarly as the preparation conditions thereof. The content of carbon atoms in the third layer (III) in the present invention is determined as desired depending on the amorphous material constituting the 50 third layer (III) and its characteristics.

More specifically, the amorphous material represented by the general formula  $a\text{-}(\text{Si}_x\text{C}_{1-x})_y(\text{H},\text{X})_{1-y}$  may be broadly classified into an amorphous material constituted of silicon atoms and carbon atoms (hereinafter referred to as "a-Si<sub>a</sub>C<sub>1-a</sub>", where  $0 < a < 1$ ), an amorphous material constituted of silicon atoms, carbon atoms and hydrogen atoms (hereinafter referred to as  $a\text{-}(\text{Si}_b\text{C}_{1-b})_c\text{H}_{1-c}$ , where  $0 < b, c < 1$ ) and an amorphous material constituted of silicon atoms, carbon atoms, 60 halogen atoms and optionally hydrogen atoms (hereinafter referred to as "a-Si<sub>d</sub>C<sub>1-d</sub>)e(H,X)<sub>1-e</sub>", where  $0 < d, e < 1$ ).

In the present invention, when the third layer (III) is to be constituted of a-Si<sub>a</sub>C<sub>1-a</sub>, the content of carbon atoms (C) in the third layer (III) may preferably be  $1 \times 10^{-3}$  to 90 atomic %, more preferably 1 to 80 atomic %, most preferably 10 to 75 atomic %, namely in terms

of representation by a, a being preferably 0.1 to 0.99999, more preferably 0.2 to 0.99, most preferably 0.25 to 0.9.

In the present invention, when the third layer (III) is to be constituted of a-Si<sub>b</sub>C<sub>1-b</sub>)<sub>c</sub>H<sub>1-c</sub>, the content of carbon atoms (C) may preferably be  $1 \times 10^{-3}$  to 90 atomic %, more preferably 1 to 90 atomic %, most preferably 10 to 80 atomic %, the content of hydrogen atoms preferably 1 to 40 atomic %, more preferably 2 to 35 atomic %, most preferably 5 to 30 atomic %, and the photoconductive member formed when the hydrogen content is within these ranges can be sufficiently applicable as excellent one in practical aspect.

That is, in terms of the representation by the above a-Si<sub>b</sub>C<sub>1-b</sub>)<sub>c</sub>H<sub>1-c</sub>, b should preferably be 0.1 to 0.99999, more preferably 0.1 to 0.99, most preferably 0.15 to 0.9, and c preferably 0.6 to 0.99, more preferably 0.65 to 0.98, most preferably 0.7 to 0.95.

When the third layer (III) is to be constituted of a-Si<sub>d</sub>C<sub>1-d</sub>)<sub>e</sub>(H,X)<sub>1-e</sub>, the content of carbon atoms may preferably be  $1 \times 10^{-3}$  to 90 atomic %, more preferably 1 to 90 atomic %, most preferably 10 to 80 atomic %, the content of halogen atoms preferably 1 to 20 atomic %, more preferably 1 to 18 atomic %, most preferably 2 to 15 atomic %. When the content of halogen atoms is within these ranges, the photoconductive member prepared is sufficiently applicable in practical aspect. The content of hydrogen atoms optionally contained may preferably be 19 atomic % or less, more preferably 13 atomic % or less.

That is, in terms of representation by d and e in the above a-Si<sub>d</sub>C<sub>1-d</sub>)<sub>e</sub>(H,X)<sub>1-e</sub>, d should preferably be 0.1 to 0.99999, more preferably 0.1 to 0.99, most preferably 0.15 to 0.9 and e preferably 0.8 to 0.99, more preferably 0.82-0.99, most preferably 0.85 to 0.98.

The range of the numerical value of layer thickness of the third layer (III) is one of the important factors to accomplish effectively the objects of the present invention. It should desirably be determined depending on the intended purpose so as to effectively accomplish the objects of the present invention.

The layer thickness of the third layer (III) is also required to be determined as desired suitably with due considerations about the relationships with the contents of carbon atoms, the relationship with the layer thicknesses of the first layer (I) and the second layer (II) as well as other organic relationships with the characteristics required for respective layer regions. In addition, it is also desirable to have considerations from economical point of view such as productivity or capability of bulk production.

The third layer (III) in the present invention is desired to have a layer thickness preferably of 0.003 to 30  $\mu\text{m}$ , more preferably 0.004 to 20  $\mu\text{m}$ , most preferably 0.005 to 10  $\mu\text{m}$ .

The substrate 101 to be used in the present invention may be either electroconductive or insulating. As the electroconductive material, there may be mentioned metals such as NiCr, stainless steel, Al, Cr, Mo, Au, Nb, Ta, V, Ti, Pt, Pd etc. or alloys thereof.

As insulating substrate, there may conventionally be used films or sheets or synthetic resins, including polyester, polyethylene, polycarbonate, cellulose acetate, polypropylene, polyvinyl chloride, polyvinylidene chloride, polystyrene, polyamide, etc., glasses, ceramics, papers and so on. These insulating substrates should preferably have at least one surface subjected to electroconductive treatment, and it is desirable to provide

other layers on the side at which said electroconductive treatment has been applied.

For example, electroconductive treatment of a glass can be effected by providing a thin film of NiCr, Al, Cr, Mo, Au, Ir, Nb, Ta, V, Ti, Pt, In<sub>2</sub>O<sub>3</sub>, SnO<sub>2</sub>, ITO (In<sub>2</sub>O<sub>3</sub> + SnO<sub>2</sub>) thereon. Alternatively, a synthetic resin film such as polyester film can be subjected to the electroconductive treatment on its surface by vacuum vapor deposition, electron-beam deposition or sputtering of a metal such as NiCr, Al, Ag, Pb, Zn, Ni, Au, Cr, Mo, Ir, Nb, Ta, V, Ti, Pt, etc. or by laminating treatment with said metal, thereby imparting electroconductivity to the surface. The substrate may be shaped in any form as desired. For example, when the photoconductive member 100 in FIG. 1 is to be used as an image forming member for electrophotography, it may desirably be formed into an endless belt or a cylinder for use in continuous high speed copying. The substrate may have a thickness, which is conveniently determined so that a photoconductive member as desired may be formed. When the photoconductive member is required to have a flexibility, the substrate is made as thin as possible, so far as the function of a substrate can be exhibited. However, in such a case, the thickness is preferably 10  $\mu$ m or more from the points of fabrication and handling of the substrate as well as its mechanical strength.

Next, an example of the process for producing the photoconductive member of this invention is to be briefly described.

FIG. 18 shows one example of a device for producing a photoconductive member according to the glow discharge decomposition method.

In the gas bombs 1102-1106 there are hermetically contained starting gases for formation of the photoconductive member of the present invention. For example, 35 1102 is a bomb containing SiH<sub>4</sub> gas diluted with He (purity: 99.999%, hereinafter abbreviated as "SiH<sub>4</sub>/He"), 1103 is a bomb containing GeH<sub>4</sub> gas diluted with He (purity: 99.999%, hereinafter abbreviated as "GeH<sub>4</sub>/He"), 1104 is a bomb containing SiF<sub>4</sub> gas diluted with He (purity: 99.99%, hereinafter abbreviated as SiF<sub>4</sub>/He gas), 1105 is a bomb containing B<sub>2</sub>H<sub>6</sub> gas diluted with He (purity: 99.999%, hereinafter abbreviated as B<sub>2</sub>H<sub>6</sub>/He) and 1106 is a bomb containing 40 C<sub>2</sub>H<sub>4</sub> gas diluted with He (purity: 99.999%, hereinafter abbreviated as C<sub>2</sub>H<sub>4</sub>/He).

Although not shown in the Figure, it is also possible to provide additional bombs other than these bombs, if necessary. For example, when oxygen atoms and/or nitrogen atoms are contained in the first layer and/or the second layer, NO gas bomb (purity: 99.99%) and NH<sub>3</sub> gas bomb (purity: 99.99%) are additionally provided.

For allowing these gases to flow into the reaction chamber 1101, on confirmation of the valves 1122-1126 of the gas bombs 1102-1106 and the leak valve 1135 being closed, and the inflow valves 1112-1116, the outflow valves 1117-1121 and the auxiliary valves 1132, 1133 being opened, the main valve 1134 is first opened to evacuate the reaction chamber 1101 and the gas pipelines. As the next step, when the reading on the vacuum indicator 1136 becomes  $5 \times 10^{-6}$  Torr, the auxiliary valves 1132, 1133 and the outflow valves 1117-1121 are closed.

Referring now to an example of forming a first layer (I) on the cylindrical substrate 1137, SiH<sub>4</sub>/He gas from the gas bomb 1102, B<sub>2</sub>H<sub>6</sub> He gas from the gas bomb

1105 are permitted to flow into the mass-flow controllers 1107, 1110, respectively, by opening the valves 1122, 1125 and controlling the pressures at the outlet pressure gauges 1127, 1130 to 1 Kg/cm<sup>2</sup> and opening gradually the inflow valves 1112, 1115, respectively. Subsequently, the outflow valves 1117, 1120 and the auxiliary valve 1132 are gradually opened to permit respective gases to flow into the reaction chamber 1101. The outflow valves 1117, 1120 are controlled so that the flow rate ratio of SiH<sub>4</sub>/He to B<sub>2</sub>H<sub>6</sub>/He may have a desired value and opening of the main valve 1134 is also controlled while watching the reading on the vacuum indicator 1136 so that the pressure in the reaction chamber may reach a desired value. After confirming that the temperature of the substrate 1137 is set at 50°-400° C. by the heater 1138, the power source 1140 is set at a desired power to excite glow discharge in the reaction chamber 1101, thereby forming a first layer (I) on the substrate cylinder 1137. For incorporating further oxygen atoms and/or nitrogen atoms in the first layer (I), NO gas and/or NH<sub>3</sub> gas may be introduced into the reaction chamber 1101, while controlling their flow rates to desired proportions relative to the flow rate of SiH<sub>4</sub>/He gas and the flow rate of B<sub>2</sub>H<sub>6</sub> gas.

During layer formation, for the purpose of uniformizing layer formation, the substrate cylinder 1137 is rotated at a constant speed by the motor 1139. Finally, all the valves of the gas operational system are closed, and the reaction chamber 1101 is evacuated one to high vacuum.

Referring next to an example of forming a second layer (II) on the thus formed first layer (I), when the reading on the vacuum indicator 1136 becomes  $5 \times 10^{-6}$  Torr, the operation similar to that as described above is repeated. That is, SiH<sub>4</sub>/He gas from the gas bomb 1102, GeH<sub>4</sub>/He gas from the gas bomb 1103 and B<sub>2</sub>H<sub>6</sub>/He gas from the gas bomb 1105 are permitted to flow into the mass flow controllers 1107, 1108 and 1110, respectively, by opening the valves 1122, 1123 and 1125, respectively to adjust the outlet pressure gauges to the pressure of 1 Kg/cm<sup>2</sup>, thereby opening gradually the in-flow valves 1112, 1113 and 1115. Subsequently, the out-flow valves 1117, 1118 and 1120, and the auxiliary valve 1132 are gradually opened to permit the respective gases into the reaction chamber 1101. The outflow valves are thereby controlled so that the ratios of SiH<sub>4</sub>/He gas flow rate, GeH<sub>4</sub>/He gas flow rate and B<sub>2</sub>H<sub>6</sub>/He gas flow rate may have desired values to control the concentration distribution of germanium atoms in the layer thickness direction in the second layer (II) to a desired distribution. Also, the opening of the main valve 1134 is controlled with watching the vacuum indicator 1136 so that the pressure in the reaction chamber may become a desired value. And, after confirming that the temperature of the substrate cylinder 1137 is set at a predetermined temperature of 50° to 400° C. by the heater 1138, the power source 1140 is set at a desired power, followed by excitation of glow discharge, thereby forming a second layer (II) on the substrate cylinder 1137 similarly as in the case of formation of the first layer (I).

When oxygen atoms and/or nitrogen atoms are to be further incorporated in the second layer (II), similarly as in the case of the first layer (I), NO gas or/and NH<sub>3</sub> gas may be introduced into the reaction chamber 1101 so that their flow rates may have desired ratios relative to other gases.

Next, when forming a third layer (III) on the thus formed second layer (II), similarly as described previously, all the valves of the gas operational system used are closed, and the reaction chamber 1101 is evacuated once to high vacuum. When the reading on the vacuum indicator 1136 becomes  $5 \times 10^{-6}$  Torr, similarly as described above, for example, by supplying SiH<sub>4</sub>/He gas from the gas bomb 1102, SiF<sub>4</sub>/He gas from the gas bomb 1104 and C<sub>2</sub>H<sub>4</sub> gas from the gas bomb 1106, glow discharge may be excited to form the third layer (III). The content of carbon atoms in the third layer (III) can be controlled by controlling the flow rate of C<sub>2</sub>H<sub>4</sub>/He gas fed.

The present invention is described by referring to the following Examples.

#### EXAMPLE 1

By means of the preparation device as shown in FIG. 18, respective samples of image forming members for electrography (96 Samples of No. 1-1A to 16-6A in total) were prepared, respectively, by forming light-receiving layers on cylinders made of aluminum according to the glow discharge method as described previously in detail under the conditions as shown in Table 1A.

The depth profiles of boron atoms and germanium atoms in respective samples are shown in FIG. 14A, FIG. 14B and in FIG. 15, respectively. The depth profiles of boron atoms and germanium atoms in respective samples were formed by controlling the gas flow rates of B<sub>2</sub>H<sub>6</sub> and GeF<sub>4</sub> by automatic operation of opening and closing of the corresponding valves following the change rate curves of the gas flow rates previously determined. Correspondence of the depth profiles of boron atoms and germanium atoms in respective samples to FIGS. 14A, 14B and 15 is listed in Table 2A.

Each of the samples thus obtained was set in a charging-exposure testing device and subjected to corona charging at  $\pm 5.0$  KV for 0.3 sec., followed immediately by irradiation of a light image. The light image was irradiated by means of a tungsten lamp light source at a dose of 0.2 lux.sec through a transmission type test chart.

Immediately thereafter,  $\ominus$  chargeable developer (containing toner and carrier) was cascaded on the surface of the image forming member to give a good toner image on the surface of the image forming member. When the toner image was transferred onto a transfer paper by corona charging of  $\pm 5.0$  KV, a clear image of high density with excellent resolution and good gradation reproducibility was obtained in every image forming member.

Then, the same experiments were repeated under the same toner image forming conditions as described above, except for using GaAs type semiconductor laser (10 mW) of 810 nm in place of the tungsten lamp as the light source, and transferred image quality was evaluated for each sample. As the result, an image of high quality, excellent in resolution and good in gradation reproducibility, could be obtained in every image forming member.

#### EXAMPLE 2

By means of the device shown in FIG. 18, respective samples of image forming members for electrophotography (48 Samples of No. 21-1A to 28-6A) were prepared, respectively, on cylindrical aluminum substrates

in the same manner as in Example 1 except for the conditions shown in Table 3A.

The depth profiles of boron atoms and germanium atoms in the light receiving layers respective samples are shown in FIG. 16 and in FIG. 17, respectively. The depth profiles of boron atoms and germanium atoms in respective samples were formed by controlling the gas flow rates of B<sub>2</sub>H<sub>6</sub> and GeF<sub>4</sub> by automatic operation of opening and closing of the corresponding valves following the change rate curves of the gas flow rates previously determined. Correspondence of the depth profiles of boron atoms and germanium atoms in respective samples to FIG. 16 and FIG. 17 is listed in Table 4A.

When image quality evaluation of the transferred toner image was performed similarly as in Example 1 by use of the thus prepared image forming member, images of high quality excellent in resolution and good in gradation reproducibility were obtained in every image forming member.

#### EXAMPLE 3

By means of the preparation device of FIG. 18, respective image forming members (24 Samples of Sample No. 12-5-1-A to 12-5-8A, 24-4-1A to 24-4-8A and 28-2-1A to 28-2-8A) were prepared following the same conditions and procedures as employed in preparation of Sample No. 12-5A in Example 1 and Samples No. 24-4A and 28-2A, in Example 2 except that the preparation conditions for the third layer (III) were changed to the respective conditions as shown in Table 5A.

By using each of the thus prepared image forming members, image quality and durability by repeated continuous usage were evaluated under the same conditions as in Example 1. The evaluation results of these respective samples are shown in Table 6A.

#### EXAMPLE 4

Except for practicing preparation of the third layer (III) and varying the target area ratio of silicon wafer to graphite during its formation to vary the content ratio of silicon atoms to carbon atoms in the third layer (III), a light-receiving layer was formed on a cylindrical aluminum substrate similarly as Sample No. 3-1A in Example 1 to prepare image forming members for electrophotography (7 Samples of Sample No. 3-1-1A to 3-1-7A).

By using each of the thus prepared image forming members, image formation, developing and cleaning steps were repeated for about 50,000 times, followed by image quality evaluation in the same manner as in Example 1 to obtain the evaluation results in Table 7A.

#### EXAMPLE 5

During formation of the third layer (III), the flow rate ratio of SiH<sub>4</sub> gas to C<sub>2</sub>H<sub>4</sub> gas was changed to vary the content ratio of silicon atoms to carbon atoms in the third layer (III), otherwise following the same procedure as Sample No. 3-1A in Example 1 to form a light-receiving layer on a cylindrical aluminum substrate, thus preparing image forming members for electrophotography (8 Samples of Sample No. 3-1-11A to 3-1-18A).

By using each of the thus prepared image forming members, image formation, developing and cleaning steps were repeated for about 50,000 times similarly as in Example 1, followed by image quality evaluation to obtain the evaluation results in Table 8A.

## EXAMPLE 6

During formation of the third layer (III), the flow rate ratios of SiH<sub>4</sub> gas, SiF<sub>4</sub> gas and C<sub>2</sub>H<sub>4</sub> gas were changed to vary the content ratio of silicon atoms to carbon atoms in the third layer (III), otherwise following the same procedure as Sample No. 301A in Example 1 to form a light-receiving layer on a cylindrical aluminum substrate, thus preparing image forming members for electrophotography (8 Samples of Sample No. 3-1-21A to 3-1-28A)

By using each of the thus prepared image forming members, image formation, developing and cleaning steps were repeated for about 50,000 times similarly as in Example 1, followed by image quality evaluation, to obtain the evaluation results shown in Table 9A.

## EXAMPLE 7

Following entirely the same procedure as in Sample No. 3-1A in Example 1, except for the layer thickness of the third layer, light-receiving layers were formed on a cylindrical aluminum substrate to prepare respective image forming members, respectively (4 Samples of Sample No. 3-1-31A to 3-1-34A).

By using each of the thus prepared image forming members, image formation, developing and cleaning steps were repeated for about 50,000 times similarly as in Example 1, followed by image quality evaluation, to obtain the evaluation results shown in Table 10A.

The common conditions of layer formation in the above Examples are shown below.

## Substrate temperature:

Formation of the first and the third layers: about 250° C.

Formation of the second layer: about 200° C.

Discharging frequency: 13.56 MHz

Inner pressure in the reaciton chamber during reaction: 0.3 Torr

## EXAMPLE 8

By means of the device for preparation of photoconductive members shown in FIG. 18, light-receiving layers were formed following the preparation conditions shown in Table 1B on aluminum cylinders according to the glow discharge decomposition method as previously described in detail to prepare respective samples of image forming members for electrophotography (960 Samples of Sample No. 1-1-1B-16-10-6B).

The depth profiles in respective samples of boron atoms contained in the layer region comprising the first layer (I) and the second layer (II) in the light-receiving layer are shown in FIG. 14A and FIG. 14B, the depth profiles of oxygen atoms in FIG. 19 and further the depth profiles of germanium atoms contained in the second layer (II) in FIG. 15.

The depth profiles of boron atoms, oxygen atoms and germanium atoms in individual samples were represented in terms of the sample No. given to respective samples.

That is, the depth profiles of boron atoms and oxygen atoms are represented by the numbers 1-1B to 16-10B as shown in Table 3B, and further the depth profiles of germanium atoms were shown by the numbers of 1 to 6 corresponding to the numbers at the end of the six kinds of depth profiles (201-206) shown in FIG. 15 annexed to the end of the numbers of 1-1-B to 16-10B shown in Table 3B.

Such depth profiles of boron atoms, oxygen atoms and germanium atoms were formed by controlling the

flow rates of B<sub>2</sub>H<sub>6</sub>/He, NO and GeF<sub>4</sub>/He gases by automatic control of opening and closing of the valves following the change rate curve of gas flow rated previously determined.

Each of the samples thus obtained was set in a charging-exposure testing device and subjected to corona charging at  $\pm 5.0$  KV for 0.3 sec., followed immediately by irradiation of a light image. The light image was irradiated by means of a tungsten lamp light source at a dose of 0.2 lux.sec through a transmission type test chart.

Immediately thereafter,  $\ominus$  chargeable developer (containing toner and carrier) was cascaded on the surface of the image forming member to give a good toner image of the surface of the image forming member. When the toner image was transferred onto a transfer paper by corona charging of  $\pm 5.0$  KV, a clear image of high density with excellent resolution and good gradation reproducibility was obtained in every image forming member.

Then, the same experiments were repeated under the same toner image forming conditions as described above, except for using GaAs type semiconductor laser (10 mW) of 810 nm in place of the tungsten lamp as the light source, and transferred image quality was evaluated for each sample. As the result, an image of high quality, excellent in resolution and good in gradation reproducibility, could be obtained in every image forming member.

## EXAMPLE 9

By means of the device for preparation of photoconductive members shown in FIG. 18, light-receiving layers were formed following the preparation conditions shown in Table 2B on aluminum cylinders according to the glow discharge decomposition method as previously described in detail to prepare respective samples of image forming members for electrophotography (432 Samples of Sample No. 21-1-1B to 28-9-6B).

The depth profiles in respective samples of boron atoms contained in the layer region comprising the first layer (I) and the second layer (II) in the light-receiving layer are shown in FIG. 16, the depth profiles of oxygen atoms in FIG. 20 and further the depth profiles of germanium atoms contained in the second layer (II) in FIG. 21.

The depth profiles of boron atoms, oxygen atoms and germanium atoms in individual samples were represented in terms of the sample No. given to respective samples similarly as in Example 8.

That is, the depth profiles of boron atoms and oxygen atoms are represented by the numbers 21-1B-28-9B as shown in Table 4B, and further the depth profiles of germanium atoms were shown by the numbers of 1 to 6 corresponding to the numbers at the end of the six kinds of depth profiles (601-606) shown in FIG. 21 annexed to the end of the numbers of 1-1B to 16-10B shown in Table 3B.

When image quality evaluation of the transferred toner image was performed under the same conditions as in Example 8 by use of the thus prepared image forming member, images of high quality excellent in resolution and good in gradation reproducibility could be obtained in every image forming member.

## EXAMPLE 10

By means of the preparation device of FIG. 18, respective image forming members (24 Samples of Sample

No. 5-5-2-1B to 5-5-2-8B, 14-10-5-1B to 14-10-5-8B, 25-3-4-1B to 25-3-4-8B) were prepared following the same conditions and procedures as employed in preparation of Sample No. 5-5-2B and 14-10-5B in Example 8 and Samples No. 25-3-4B in Example 9, except that the preparation conditions for the third layer (III) were changed to the respective conditions as shown in Table 5B.

By using each of the thus prepared image forming members, image quality and durability by repeated continuous use were evaluated under the same conditions as in Example 8. The evaluation results of these respective samples are shown in Table 6B.

#### EXAMPLE 11

Except for practicing preparation of the third layer (III) and varying variously the target area ratio of silicon wafer to graphite during its formation to vary the content ratio of silicon atoms to carbon atoms in the third layer (III), a light-receiving layer was formed on a cylindrical aluminum substrate similarly as Sample No. 8-9-4B in Example 8 to prepare image forming members for electrophotography (7 Samples of Sample No. 8-9-4-1B to 8-9-4-7B).

By using each of the thus prepared image forming members, image formation, developing and cleaning steps were repeated for about 50,000 times, followed by image quality evaluation in the same manner as in Example 8 to obtain the evaluation results in Table 7B.

During formation of the third layer (III), the flow rate ratio of SiH<sub>4</sub> gas to C<sub>2</sub>H<sub>4</sub> gas was changed to vary the content ratio of silicon atoms to carbon atoms in the third layer (III), otherwise following the same procedure as Sample No. 8-9-4B in Example 8 to form a light-receiving layer on a cylindrical aluminum substrate, thus preparing image forming members for electrophotography (8 Samples of Sample No. 8-9-4-11B to 8-9-4-18B).

By using each of the thus prepared image forming members, image formation, developing and cleaning steps were repeated for about 50,000 times similarly as in Example 8, followed by image quality evaluation to obtain the evaluation results in Table 8B.

#### EXAMPLE 13

During formation of the third layer (III), the flow rate ratios of SiH<sub>4</sub> gas, SiF<sub>4</sub> gas and C<sub>2</sub>H<sub>4</sub> gas were changed to vary the content ratio of silicon atoms to carbon atoms in the third layer (III), otherwise following the same procedure as Sample No. 8-9-4B in Example 8 to form a light-receiving layer on a cylindrical aluminum substrate, thus preparing image forming members for electrophotography (8 Samples of Sample No. 8-9-4-21B to 8-9-4-28B).

By using each of the thus prepared image forming members, image formation, developing and cleaning steps were repeated for about 50,000 times similarly as in Example 8, followed by image quality evaluation to obtain the evaluation results in Table 9B.

#### EXAMPLE 14

Following entirely the same procedure as in Sample No. 8-9-4B in Example 8, except for the layer thickness of the third layer, light-receiving layer was formed on a cylindrical aluminum substrate to prepare respective image forming members, respectively (4 Samples of Sample No. 8-9-4-31B to 8-9-4-34B).

By using each of the thus prepared image forming members, image formation, developing and cleaning steps were repeated for about 50,000 times similarly as in Example 8, followed by image quality evaluation, to obtain the evaluation results shown in Table 10B.

The common conditions of layer formation in the above Examples are shown below.

Substrate temperature:

Formation of the first and the third layers: about 250° C.

Formation of the second layer: about 200° C.

Discharging frequency: 13.56 MHz

Inner pressure in the reaction chamber during reaction: 0.3 Torr

#### EXAMPLE 15

By means of the device for preparation of photoconductive members shown in FIG. 18, light-receiving layers were formed following the preparation conditions shown in Table 1C on aluminum cylinders according to the glow discharge decomposition method as previously described in detail to prepare respective samples of image forming members for electrophotography (960 Samples of Sample No. 1-1-1C to 16-10-6C).

The depth profiles in respective samples of boron atoms contained in the layer region comprising the first layer (I) and the second layer (II) in the light-receiving layer are shown in FIG. 14A and FIG. 14B, the depth profiles of nitrogen atoms in FIG. 22 and further the depth profiles of germanium atoms contained in the second layer (II) in FIG. 15.

The depth profiles of boron atoms, nitrogen atoms and germanium atoms in individual samples were represented in terms of the sample No. given to respective samples.

That is, the depth profiles of boron atoms and nitrogen atoms are represented by the numbers 1-1C to 16-10C as shown in Table 3C, and further the depth profiles of germanium atoms were shown by the numbers of 1 to 6 corresponding to the numbers at the end of the six kinds of depth profiles (201-206) shown in FIG. 15 annexed to the end of the numbers of 1-1C to 16-10C shown in Table 3C.

Such depth profiles of boron atoms, nitrogen atoms and germanium atoms were formed by controlling the flow rates of B<sub>2</sub>H<sub>6</sub>/He, NH<sub>3</sub> and GeF<sub>4</sub>/He gases by automatic control of opening and closing of the valves following the change rate curves of gas flow rates previously determined.

Each of the samples thus obtained was set in a charging-exposure testing device and subjected to corona charging at  $\pm 5.0$  KV for 0.3 sec., followed immediately by irradiation of a light image. The light image was irradiated by means of a tungsten lamp light source at a dose of 0.2 lux.sec through a transmission type test chart.

Immediately thereafter,  $\Theta$ chargeable developer (containing toner and carrier) was cascaded on the surface of the image forming member to give a good toner image of the surface of the image forming member. When the toner image was transferred onto a transfer paper by corona charging of  $\pm 5.0$  KV, a clear image of high density with excellent resolution and good gradation reproducibility was obtained in every image forming member.

Then, the same experiments were repeated under the same toner image forming conditions as described above, except for using GaAs type semiconductor laser (10 mW) of 810 nm in place of the tungsten lamp as the

light source, and image quality evaluation was performed for each sample. As the result, an image of high quality, excellent in resolution and good in gradation reproducibility, could be obtained in every image forming member.

#### EXAMPLE 16

By means of the device for preparation of photoconductive members shown in FIG. 18, light-receiving layers were formed in the same manner as in Example 15, on aluminum cylinders except for the preparation conditions shown in Table 2C to prepare respective samples of image forming members for electrophotography (432 Samples of Sample No. 21-1-1C-28-9-6C).

The depth profiles in respective samples of boron atoms contained in the layer region comprising the first layer (I) and the second layer (II) in the light-receiving layer are shown in FIG. 16, the depth profiles of nitrogen atoms in FIG. 23 and further the depth profiles of germanium atoms contained in the second layer (II) in FIG. 24.

The depth profiles of boron atoms, nitrogen atoms and germanium atoms in individual samples were represented in terms of the sample No. affixed to respective samples similarly as in Example 15.

That is, the depth profiles of boron atoms and nitrogen atoms are represented by the numbers 21-1C-28-9C as shown in Table 4C, and further the depth profiles of germanium atoms were shown by the numbers of 1 to 6 corresponding to the numbers at the end of the six kinds of depth profiles (601C-606C) shown in FIG. 24 annexed to the end of the numbers of 1-1C-16-10C shown in Table 3C.

When image quality evaluation of the transferred toner image was performed under the same conditions as in Example 15 by use of the thus prepared image forming member, images of high quality excellent in resolution and good in gradation reproducibility could be obtained in every image forming member.

#### EXAMPLE 17

By means of the preparation device of FIG. 18, respective image forming members (24 Samples of Sample No. 5-5-2-1C-5-5-2-8C, 14-10-5-1C-14-10-5-8C, 25-3-4-1C-25-3-4-8C were prepared following the same conditions and procedures as employed in preparation of Sample No. 5-5-2C and 14-10-5C in Example 15 and Samples No. 25-3-4C in Example 16, except that the preparation conditions for the third layer (III) were changed to the respective conditions as shown in Table 5C.

By using each of the thus prepared image forming members, image quality and durability by repeated continuous usage were evaluated under the same conditions as in Example 15. The evaluation results of these respective samples are shown in Table 6C.

#### EXAMPLE 18

Except for practicing preparation of the third layer (III) and varying the target area ratio of silicon wafer to graphite during its formation to vary the content ratio of silicon atoms to carbon atoms in the third layer (III), a light-receiving layer was formed on a cylindrical alu-

minum substrate similarly as Sample No. 8-9-4C in Example 15 to prepare image forming members for electrophotography (7 Samples of Sample No. 8-9-4-1C-8-9-4-7C).

By using each of the thus prepared image forming members, image formation, developing and cleaning steps were repeated for about 50,000 times similarly as in Example 15, followed by image quality evaluation to obtain the evaluation results in Table 7C.

#### EXAMPLE 19

During formation of the third layer (III), the flow rate ratio of SiH<sub>4</sub> gas to C<sub>2</sub>H<sub>4</sub> gas was changed to vary the content ratio of silicon atoms to carbon atoms in the third layer (III), otherwise following the same procedure as Sample No. 8-9-4C in Example 15 to form a light-receiving layer on a cylindrical aluminum substrate, thus preparing image forming members for electrophotography (8 Samples of Sample No. 8-9-4-11C to 8-9-4-18C).

By using each of the thus prepared image forming members, image formation, developing and cleaning steps were repeated for about 50,000 times similarly as in Example 15, followed by image quality evaluation to obtain the evaluation results in Table 8C.

#### EXAMPLE 20

During formation of the third layer (III), the flow rate ratios of SiH<sub>4</sub> gas, SiF<sub>4</sub> gas and C<sub>2</sub>H<sub>4</sub> gas were changed to vary the content ratio of silicon atoms to carbon atoms in the third layer (III), otherwise following the same procedure as Sample No. 8-9-4C in Example 15 to form a light-receiving layer on a cylindrical aluminum substrate, thus preparing image forming members for electrophotography (8 Samples of Sample No. 8-9-4-21C to 8-9-4-28C).

By using each of the thus prepared image forming members, image formation, developing and cleaning steps were repeated for about 50,000 times similarly as in Example 15, followed by image quality evaluation to obtain the evaluation results in Table 9C.

#### EXAMPLE 21

Following entirely the same procedure as in Sample No. 8-9-4C in Example 15, except for varying the layer thickness of the third layer, light-receiving layer was formed on a cylindrical aluminum substrate to prepare respective image forming members, respectively (4 Samples of Sample No. 8-9-4-31C to 8-9-4-34C).

By using each of the thus prepared image forming members, image formation, developing and cleaning steps were repeated for about 50,000 times similarly as in Example 15, followed by image quality evaluation, to obtain the evaluation results shown in Table 10C.

The common layer forming conditions in the above Examples are shown below.

Substrate temperature:

Formation of the first and the third layers: about 250° C.

Formation of the second layer: about 200° C.

Discharging frequency: 13.56 MHz

Inner pressure in the reaction chamber during reaction:

0.3 Torr

TABLE 1A

| Layer<br>Constitu-<br>tion | Gases<br>employed                                                                                                                  | Flow rate<br>(SCCM)                       | Flow rate ratio                                       | Dis-<br>charging<br>power<br>(W/cm <sup>2</sup> ) | Layer<br>formation<br>rate<br>(Å/sec) | Layer<br>thick-<br>ness<br>(μm) |
|----------------------------|------------------------------------------------------------------------------------------------------------------------------------|-------------------------------------------|-------------------------------------------------------|---------------------------------------------------|---------------------------------------|---------------------------------|
| First<br>layer<br>(I)      | SiH <sub>4</sub> /He = 0.5<br>B <sub>2</sub> H <sub>6</sub> /Ge = 10 <sup>-3</sup>                                                 | SiH <sub>4</sub> = 200                    |                                                       | 0.18                                              | 15                                    | 5                               |
| Second<br>layer<br>(II)    | SiF <sub>4</sub> /He = 0.5<br>GeF <sub>4</sub> /He = 0.5<br>H <sub>2</sub><br>B <sub>2</sub> H <sub>6</sub> /He = 10 <sup>-3</sup> | SiF <sub>4</sub> + GeF <sub>4</sub> = 200 |                                                       | 0.18                                              | 15                                    | 20                              |
| Third<br>layer<br>(III)    | SiH <sub>4</sub> /He = 0.5<br>C <sub>2</sub> H <sub>4</sub>                                                                        | SiH <sub>4</sub> = 100                    | SiH <sub>4</sub> /C <sub>2</sub> H <sub>4</sub> = 3/7 | 0.18                                              | 10                                    | 0.5                             |

TABLE 2A

| Depth profile<br>No. of boron | Sample No. | Depth profile No. of germanium |       |       |       |       |       |
|-------------------------------|------------|--------------------------------|-------|-------|-------|-------|-------|
|                               |            | 201                            | 202   | 203   | 204   | 205   | 206   |
| 101                           |            | 1-1A                           | 1-2A  | 1-3A  | 1-4A  | 1-5A  | 1-6A  |
| 102                           |            | 2-1A                           | 2-2A  | 2-3A  | 2-4A  | 2-5A  | 2-6A  |
| 103                           |            | 3-1A                           | 3-2A  | 3-3A  | 3-4A  | 3-5A  | 3-6A  |
| 104                           |            | 4-1A                           | 4-2A  | 4-3A  | 4-4A  | 4-5A  | 4-6A  |
| 105                           |            | 5-1A                           | 5-2A  | 5-3A  | 5-4A  | 5-5A  | 5-6A  |
| 106                           |            | 6-1A                           | 6-2A  | 6-3A  | 6-4A  | 6-5A  | 6-6A  |
| 107                           |            | 7-1A                           | 7-2A  | 7-3A  | 7-4A  | 7-5A  | 7-6A  |
| 108                           |            | 8-1A                           | 8-2A  | 8-3A  | 8-4A  | 8-5A  | 8-6A  |
| 109                           |            | 9-1A                           | 9-2A  | 9-3A  | 9-4A  | 9-5A  | 9-6A  |
| 110                           |            | 10-1A                          | 10-2A | 10-3A | 10-4A | 10-5A | 10-6A |
| 111                           |            | 11-1A                          | 11-2A | 11-3A | 11-4A | 11-5A | 11-6A |
| 112                           |            | 12-1A                          | 12-2A | 12-3A | 12-4A | 12-5A | 12-6A |
| 113                           |            | 13-1A                          | 13-2A | 13-3A | 13-4A | 13-5A | 13-6A |
| 114                           |            | 14-1A                          | 14-2A | 14-3A | 14-4A | 14-5A | 14-6A |
| 115                           |            | 15-1A                          | 15-2A | 15-3A | 15-4A | 15-5A | 15-6A |
| 116                           |            | 16-1A                          | 16-2A | 16-3A | 16-4A | 16-5A | 16-6A |

TABLE 3A

| Layer<br>Constitu-<br>tion | Gases<br>employed                                                                                                                  | Flow rate<br>(SCCM)                       | Flow rate ratio                                       | Dis-<br>charging<br>power<br>(W/cm <sup>2</sup> ) | Layer<br>formation<br>rate<br>(Å/sec) | Layer<br>thick-<br>ness<br>(μm) |
|----------------------------|------------------------------------------------------------------------------------------------------------------------------------|-------------------------------------------|-------------------------------------------------------|---------------------------------------------------|---------------------------------------|---------------------------------|
| First<br>layer<br>(I)      | SiH <sub>4</sub> /He = 0.5<br>B <sub>2</sub> H <sub>6</sub> /He = 10 <sup>-3</sup>                                                 | SiH <sub>4</sub> = 200                    |                                                       | 0.18                                              | 15                                    | 20                              |
| Second<br>layer<br>(II)    | SiF <sub>4</sub> /He = 0.5<br>GeF <sub>4</sub> /He = 0.5<br>H <sub>2</sub><br>B <sub>2</sub> H <sub>6</sub> /He = 10 <sup>-3</sup> | SiF <sub>4</sub> + GeF <sub>4</sub> = 200 |                                                       | 0.18                                              | 15                                    | 5                               |
| Third<br>layer<br>(III)    | SiH <sub>4</sub> /He = 0.5<br>C <sub>2</sub> H <sub>4</sub>                                                                        | SiH <sub>4</sub> = 100                    | SiH <sub>4</sub> /C <sub>2</sub> H <sub>4</sub> = 3/7 | 0.18                                              | 10                                    | 0.5                             |

TABLE 4A

| Depth profile<br>No. of boron | Sample No. | Depth profile No. of germanium |       |       |       |       |       |
|-------------------------------|------------|--------------------------------|-------|-------|-------|-------|-------|
|                               |            | 401                            | 402   | 403   | 404   | 405   | 406   |
| 301                           |            | 21-1A                          | 21-2A | 21-3A | 21-4A | 21-5A | 21-6A |
| 302                           |            | 22-1A                          | 22-2A | 22-3A | 22-4A | 22-5A | 22-6A |
| 303                           |            | 23-1A                          | 23-2A | 23-3A | 23-4A | 23-5A | 24-6A |
| 304                           |            | 24-1A                          | 24-2A | 24-3A | 24-4A | 24-5A | 24-6A |
| 305                           |            | 25-1A                          | 25-2A | 25-3A | 25-4A | 25-5A | 25-6A |
| 306                           |            | 26-1A                          | 26-2A | 26-3A | 26-4A | 26-5A | 26-6A |
| 307                           |            | 27-1A                          | 27-2A | 27-3A | 27-4A | 27-5A | 27-6A |
| 308                           |            | 28-1A                          | 28-2A | 28-3A | 28-4A | 28-5A | 28-6A |

TABLE 5A

| Condi-<br>tions | Gases<br>employed | Flow rate<br>(SCCM) | Flow rate ratio<br>or Area ratio | Discharging<br>power<br>(W/cm <sup>2</sup> ) | Layer<br>thickness<br>(μm) |
|-----------------|-------------------|---------------------|----------------------------------|----------------------------------------------|----------------------------|
| 1               | Ar                | 200                 | Si wafer:graphite = 1.5:9.5      | 0.3                                          | 0.5                        |
| 2               | Ar                | 200                 | Si wafer:graphite = 1.5:9.5      | 0.3                                          | 0.3                        |

TABLE 5A-continued

| Condi-<br>tions | Gases<br>employed                                                                         | Flow rate<br>(SCCM)                                                                                      | Flow rate ratio<br>or Area ratio                                                | Discharging<br>power<br>(W/cm <sup>2</sup> ) | Layer<br>thickness<br>(μm) |
|-----------------|-------------------------------------------------------------------------------------------|----------------------------------------------------------------------------------------------------------|---------------------------------------------------------------------------------|----------------------------------------------|----------------------------|
| 3               | Ar                                                                                        | 200                                                                                                      | Si wafer:graphite =<br>1.5:9.5                                                  | 0.3                                          | 1.0                        |
| 4               | SiH <sub>4</sub> /He = 1<br>C <sub>2</sub> H <sub>4</sub>                                 | SiH <sub>4</sub> = 150                                                                                   | SiH <sub>4</sub> :C <sub>2</sub> H <sub>4</sub> = 5:5                           | 0.18                                         | 0.3                        |
| 5               | SiH <sub>4</sub> /He = 0.5<br>C <sub>2</sub> H <sub>4</sub>                               | SiH <sub>4</sub> = 100                                                                                   | SiH <sub>4</sub> :C <sub>2</sub> H <sub>4</sub> = 5:5                           | 0.18                                         | 1.5                        |
| 6               | SiH <sub>4</sub> /He = 0.5<br>SiF <sub>4</sub> /He = 0.5<br>C <sub>2</sub> H <sub>4</sub> | SiH <sub>4</sub> + SiF <sub>4</sub> = 150<br>SiF <sub>4</sub> /He = 0.5<br>C <sub>2</sub> H <sub>4</sub> | SiH <sub>4</sub> :SiF <sub>4</sub> :C <sub>2</sub> H <sub>4</sub> = 1.5:1.5:7   | 0.18                                         | 0.5                        |
| 7               | SiH <sub>4</sub> /He = 0.5<br>SiF <sub>4</sub> /He = 0.5<br>C <sub>2</sub> H <sub>4</sub> | SiH <sub>4</sub> + SiF <sub>4</sub> = 150<br>SiF <sub>4</sub> /He = 0.5<br>C <sub>2</sub> H <sub>4</sub> | SiH <sub>4</sub> :SiF <sub>4</sub> :C <sub>2</sub> H <sub>4</sub> = 0.3:0.1:9.6 | 0.18                                         | 0.3                        |
| 8               | SiH <sub>4</sub> /He = 0.5<br>SiF <sub>4</sub> /He = 0.5<br>C <sub>2</sub> H <sub>4</sub> | SiH <sub>4</sub> + SiF <sub>4</sub> = 150<br>SiF <sub>4</sub> /He = 0.5<br>C <sub>2</sub> H <sub>4</sub> | SiH <sub>4</sub> :SiF <sub>4</sub> :C <sub>2</sub> H <sub>4</sub> = 3:3:4       | 0.18                                         | 1.5                        |

TABLE 6A

20

TABLE 6A-continued

| Layer (III)<br>forming<br>conditions | Sample No./Evaluation |                |                | Sample No.     | Overall image<br>quality<br>evaluation | Durability<br>evaluation | Evaluation standards:<br>◎: Excellent<br>○: Good |
|--------------------------------------|-----------------------|----------------|----------------|----------------|----------------------------------------|--------------------------|--------------------------------------------------|
|                                      | 1                     | 12-5-1A<br>○ ○ | 24-4-1A<br>○ ○ | 28-2-1A<br>○ ○ |                                        |                          |                                                  |
| 2                                    | 12-5-2A<br>○ ○        | 24-4-2A<br>○ ○ | 28-2-2A<br>○ ○ | 25             | 6<br>○ ○                               | 12-5-6A<br>○ ○           | 24-4-6A<br>○ ○                                   |
| 3                                    | 12-5-3A<br>○ ○        | 24-4-3A<br>○ ○ | 28-2-3A<br>○ ○ |                | 7<br>○ ○                               | 12-5-7A<br>○ ○           | 24-4-7A<br>○ ○                                   |
| 4                                    | 12-5-4A<br>○ ○        | 24-4-4A<br>○ ○ | 28-2-4A<br>○ ○ |                | 8<br>○ ○                               | 12-5-8A<br>○ ○           | 24-4-8A<br>○ ○                                   |
| 5                                    | 12-5-5A<br>○ ○        | 24-4-5A<br>○ ○ | 28-2-5A<br>○ ○ | 30             |                                        |                          | 28-2-6A<br>○ ○                                   |

TABLE 7A

| Sample No.                     | 3-1-1A  | 3-1-2A  | 3-1-3A  | 3-1-4A  | 3-1-5A | 3-1-6A  | 3-1-7A  |
|--------------------------------|---------|---------|---------|---------|--------|---------|---------|
| Si:C<br>Target<br>Area ratio   | 9:1     | 6.5:3.5 | 4:6     | 2:8     | 1:9    | 0.5:9.5 | 0.2:9.8 |
| Si:C<br>(Content<br>ratio)     | 9.7:0.3 | 8.8:1.2 | 7.3:2.7 | 4.8:5.2 | 3:7    | 2:8     | 0.8:9.2 |
| Image<br>quality<br>evaluation | Δ       | ○       | ◎       | ○       | Δ      | Δ       | X       |

◎: Very good

○: Good

Δ: Sufficiently practically usable

X: Image defect formed

TABLE 8A

| Sample No.                                               | 3-1-11A | 3-1-12A | 3-1-13A | 3-1-14A | 3-1-15A | 3-1-16A | 3-1-17A   | 3-1-18A |
|----------------------------------------------------------|---------|---------|---------|---------|---------|---------|-----------|---------|
| Si:C <sub>2</sub> H <sub>4</sub><br>(Flow rate<br>ratio) | 9:1     | 6:4     | 4:6     | 2:8     | 1:9     | 0.5:9.5 | 0.35:9.65 | 0.2:9.8 |
| Si:C<br>(Content<br>ratio)                               | 9:1     | 7:3     | 5.5:4.5 | 4:6     | 3:7     | 2:8     | 1.2:8.8   | 0.8:9.2 |
| Image<br>quality<br>evaluation                           | Δ       | ○       | ◎       | ○       | ◎       | ○       | Δ         | X       |

◎: Very good

○: Good

Δ: Sufficiently practically usable

X: Image defect formed

TABLE 9A

| Sample No.                                                                                | 3-1-21A | 3-1-22A   | 3-1-23A | 3-1-24A | 3-1-25A   | 3-1-26A     | 3-1-27A       | 3-1-28A     |
|-------------------------------------------------------------------------------------------|---------|-----------|---------|---------|-----------|-------------|---------------|-------------|
| SiH <sub>4</sub> :SiF <sub>4</sub> :C <sub>2</sub> H <sub>4</sub><br>(Flow rate<br>ratio) | 5:4:1   | 3:3.5:3.5 | 2:2.6   | 1:1:8   | 0.6:0.4:9 | 0.2:0.3:9.5 | 0.2:0.15:9.65 | 0.1:0.1:9.8 |
| Si:C<br>(Content<br>ratio)                                                                | 9:1     | 7:3       | 5.5:4.5 | 4:6     | 3:7       | 2:8         | 1.2:8.8       | 0.8:9.2     |
| Image                                                                                     | Δ       | ○         | ◎       | ○       | ◎         | ○           | Δ             | X           |

TABLE 9A-continued

| Sample No. | 3-1-21A | 3-1-22A | 3-1-23A | 3-1-24A | 3-1-25A | 3-1-26A | 3-1-27A | 3-1-28A |
|------------|---------|---------|---------|---------|---------|---------|---------|---------|
|------------|---------|---------|---------|---------|---------|---------|---------|---------|

quality  
evaluation

○: Very good  
◎: Good  
△: Sufficiently practically usable  
×: Image defect formed

TABLE 10A

10

TABLE 10A-continued

| Sample No. | Thickness of layer (III) (μm) | Results                                                          | Sample No. | Thickness of layer (III) (μm) | Results                                          |
|------------|-------------------------------|------------------------------------------------------------------|------------|-------------------------------|--------------------------------------------------|
| 3-1-31A    | 0.001                         | Image defect liable to occur                                     | 3-1-33A    | 0.05                          | Stable up to successive copying for 50,000 times |
| 3-1-32A    | 0.02                          | No image defect formed up to successive copying for 20,000 times | 15         | 3-1-34A                       | 1                                                |

TABLE 1B

| Layer constitution | Gases employed                                                                                                                           | Flow rate (SCCM)                          | Flow rate ratio                                       | Discharging power (W/cm <sup>2</sup> ) | Layer formation rate (Å/sec) | Layer thickness (μm) |
|--------------------|------------------------------------------------------------------------------------------------------------------------------------------|-------------------------------------------|-------------------------------------------------------|----------------------------------------|------------------------------|----------------------|
| First layer (I)    | SiH <sub>4</sub> /He = 0.5<br>B <sub>2</sub> H <sub>6</sub> /He = 10 <sup>-3</sup><br>NO                                                 | SiH <sub>4</sub> = 200                    |                                                       | 0.18                                   | 15                           | 5                    |
| Second layer (II)  | SiF <sub>4</sub> /He = 0.5<br>GeF <sub>4</sub> /He = 0.5<br>B <sub>2</sub> H <sub>6</sub> /He = 10 <sup>-3</sup><br>H <sub>2</sub><br>NO | SiF <sub>4</sub> + GeF <sub>4</sub> = 200 |                                                       | 0.18                                   | 15                           | 20                   |
| Third layer (III)  | SiH <sub>4</sub> /He = 0.5<br>C <sub>2</sub> H <sub>4</sub>                                                                              | SiH <sub>4</sub> = 100                    | SiH <sub>4</sub> /C <sub>2</sub> H <sub>4</sub> = 3/7 | 0.18                                   | 10                           | 0.5                  |

TABLE 2B

| Layer constitution | Gases employed                                                                                                                           | Flow rate (SCCM)                          | Flow rate ratio                                       | Discharging power (W/cm <sup>2</sup> ) | Layer formation rate (Å/sec) | Layer thickness (μm) |
|--------------------|------------------------------------------------------------------------------------------------------------------------------------------|-------------------------------------------|-------------------------------------------------------|----------------------------------------|------------------------------|----------------------|
| First layer (I)    | SiH <sub>4</sub> /He = 0.5<br>B <sub>2</sub> H <sub>6</sub> /He = 10 <sup>-3</sup><br>NO                                                 | SiH <sub>4</sub> = 200                    |                                                       | 0.18                                   | 15                           | 20                   |
| Second layer (II)  | SiF <sub>4</sub> /He = 0.5<br>GeF <sub>4</sub> /He = 0.5<br>B <sub>2</sub> H <sub>6</sub> /He = 10 <sup>-3</sup><br>H <sub>2</sub><br>NO | SiF <sub>4</sub> + GeF <sub>4</sub> = 200 |                                                       | 0.18                                   | 15                           | 5                    |
| Third layer (III)  | SiH <sub>4</sub> /He = 0.5<br>C <sub>2</sub> H <sub>4</sub>                                                                              | SiH <sub>4</sub> = 100                    | SiH <sub>4</sub> /C <sub>2</sub> H <sub>4</sub> = 3/7 | 0.18                                   | 10                           | 0.5                  |

TABLE 3B

| Depth profile No. of boron | Sample No. | Depth profile No. of oxygen |       |       |       |       |       |       |       |       |        |
|----------------------------|------------|-----------------------------|-------|-------|-------|-------|-------|-------|-------|-------|--------|
|                            |            | 201B                        | 202B  | 203B  | 204B  | 205B  | 206B  | 207B  | 208B  | 209B  | 210B   |
| 101                        |            | 1-1B                        | 1-2B  | 1-3B  | 1-4B  | 1-5B  | 1-6B  | 1-7B  | 1-8B  | 1-9B  | 1-10B  |
| 102                        |            | 2-1B                        | 2-2B  | 2-3B  | 2-4B  | 2-5B  | 2-6B  | 2-7B  | 2-8B  | 2-9B  | 2-10B  |
| 103                        |            | 3-1B                        | 3-2B  | 3-3B  | 3-4B  | 3-5B  | 3-6B  | 3-7B  | 3-8B  | 3-9B  | 3-10B  |
| 104                        |            | 4-1B                        | 4-2B  | 4-3B  | 4-4B  | 4-5B  | 4-6B  | 4-7B  | 4-8B  | 4-9B  | 4-10B  |
| 105                        |            | 5-1B                        | 5-2B  | 5-3B  | 5-4B  | 5-5B  | 5-6B  | 5-7B  | 5-8B  | 5-9B  | 5-10B  |
| 106                        |            | 6-1B                        | 6-2B  | 6-3B  | 6-4B  | 6-5B  | 6-6B  | 6-7B  | 6-8B  | 6-9B  | 6-10B  |
| 107                        |            | 7-1B                        | 7-2B  | 7-3B  | 7-4B  | 7-5B  | 7-6B  | 7-7B  | 7-8B  | 7-9B  | 7-10B  |
| 108                        |            | 8-1B                        | 8-2B  | 8-3B  | 8-4B  | 8-5B  | 8-6B  | 8-7B  | 8-8B  | 8-9B  | 8-10B  |
| 109                        |            | 9-1B                        | 9-2B  | 9-3B  | 9-4B  | 9-5B  | 9-6B  | 9-7B  | 9-8B  | 9-9B  | 9-10B  |
| 110                        |            | 10-1B                       | 10-2B | 10-3B | 10-4B | 10-5B | 10-6B | 10-7B | 10-8B | 10-9B | 10-10B |
| 111                        |            | 11-1B                       | 11-2B | 11-3B | 11-4B | 11-5B | 11-6B | 11-7B | 11-8B | 11-9B | 11-10B |
| 112                        |            | 12-1B                       | 12-2B | 12-3B | 12-4B | 12-5B | 12-6B | 12-7B | 12-8B | 12-9B | 12-10B |
| 113                        |            | 13-1B                       | 13-2B | 13-3B | 13-4B | 13-5B | 13-6B | 13-7B | 13-8B | 13-9B | 13-10B |
| 114                        |            | 14-1B                       | 14-2B | 14-3B | 14-4B | 14-5B | 14-6B | 14-7B | 14-8B | 14-9B | 14-10B |
| 115                        |            | 15-1B                       | 15-2B | 15-3B | 15-4B | 15-5B | 15-6B | 15-7B | 15-8B | 15-9B | 15-10B |
| 116                        |            | 16-1B                       | 16-2B | 16-3B | 16-4B | 16-5B | 16-6B | 16-7B | 16-8B | 16-9B | 16-10B |



TABLE 8B-continued

Sample No. 8-9-4-11B 8-9-4-12B 8-9-4-13B 8-9-4-14B 8-9-4-15B 8-9-4-16B 8-9-4-17B 8-9-4-18B

quality  
evaluation

◎: Very good

○: Good

△: Sufficiently practically usable

X: Image defect formed

TABLE 9B

Sample No. 8-9-4-21B 8-9-4-22B 8-9-4-23B 8-9-4-24B 8-9-4-25B 8-9-4-26B 8-9-4-27B 8-9-4-28B

SiH<sub>4</sub>:SiF<sub>4</sub>:C<sub>2</sub>H<sub>4</sub> 5:4:1 3:3.5:3.5 2:2:6 1:1:8 0.6:0.4:9 0.2:0.3:9.5 0.2:0.15:9.65 0.1:0.1:9.8  
(Flow rate  
ratio)Si:C 9:1 7:3 5.5:4.5 4:6 3:7 2:8 1.2:8.8 0.8:9.2  
(Content  
ratio)Image  
quality  
evaluation

◎: Very good

○: Good

△: Sufficiently practically usable

X: Image defect formed

TABLE 10B

| Sample No. | Thickness of<br>layer (III) (μm) | Results                                                                |
|------------|----------------------------------|------------------------------------------------------------------------|
| 8-9-4-31B  | 0.001                            | Image defect liable<br>to occur                                        |
| 8-9-4-32B  | 0.02                             | No image defect formed<br>up to successive copying<br>for 20,000 times |

TABLE 10B-continued

| Sample No. | Thickness of<br>layer (III) (μm) | Results                                                 |
|------------|----------------------------------|---------------------------------------------------------|
| 8-9-4-33B  | 0.05                             | Stable up to successive<br>copying for 50,000 times     |
| 8-9-4-34B  | 1                                | Stable up to successive<br>copying for 200,000<br>times |

TABLE 1C

| Layer<br>consti-<br>tution | Gases<br>employed                                                                                                                                     | Flow rate<br>(SCCM)                       | Flow rate ratio                                       | Dis-<br>charging<br>power<br>(W/cm <sup>2</sup> ) | Layer<br>formation<br>rate<br>(Å/sec) | Layer<br>thick-<br>ness<br>(μm) |
|----------------------------|-------------------------------------------------------------------------------------------------------------------------------------------------------|-------------------------------------------|-------------------------------------------------------|---------------------------------------------------|---------------------------------------|---------------------------------|
| First<br>layer<br>(I)      | SiH <sub>4</sub> /He = 0.5<br>B <sub>2</sub> H <sub>6</sub> /He = 10 <sup>-3</sup><br>NH <sub>3</sub>                                                 | SiH <sub>4</sub> = 200                    |                                                       | 0.18                                              | 15                                    | 5                               |
| Second<br>layer<br>(II)    | SiF <sub>4</sub> /He = 0.5<br>GeF <sub>4</sub> /He = 0.5<br>B <sub>2</sub> H <sub>6</sub> /He = 10 <sup>-3</sup><br>H <sub>2</sub><br>NH <sub>3</sub> | SiF <sub>4</sub> + GeF <sub>4</sub> = 200 |                                                       | 0.18                                              | 15                                    | 20                              |
| Third<br>layer<br>(III)    | SiH <sub>4</sub> /He = 0.5<br>C <sub>2</sub> H <sub>4</sub>                                                                                           | SiH <sub>4</sub> = 100                    | SiH <sub>4</sub> /C <sub>2</sub> H <sub>4</sub> = 3/7 | 0.18                                              | 10                                    | 0.5                             |

TABLE 2C

| Layer<br>consti-<br>tution | Gases<br>employed                                                                                                                                     | Flow rate<br>(SCCM)                       | Flow rate ratio                                       | Dis-<br>charging<br>power<br>(W/cm <sup>2</sup> ) | Layer<br>formation<br>rate<br>(Å/sec) | Layer<br>thick-<br>ness<br>(μm) |
|----------------------------|-------------------------------------------------------------------------------------------------------------------------------------------------------|-------------------------------------------|-------------------------------------------------------|---------------------------------------------------|---------------------------------------|---------------------------------|
| First<br>layer<br>(I)      | SiH <sub>4</sub> /He = 0.5<br>B <sub>2</sub> H <sub>6</sub> /He = 10 <sup>-3</sup><br>NH <sub>3</sub>                                                 | SiH <sub>4</sub> = 200                    |                                                       | 0.18                                              | 15                                    | 20                              |
| Second<br>layer<br>(II)    | SiF <sub>4</sub> /He = 0.5<br>GeF <sub>4</sub> /He = 0.5<br>B <sub>2</sub> H <sub>6</sub> /He = 10 <sup>-3</sup><br>H <sub>2</sub><br>NH <sub>3</sub> | SiF <sub>4</sub> + GeF <sub>4</sub> = 200 |                                                       | 0.18                                              | 15                                    | 5                               |
| Third<br>layer<br>(III)    | SiH <sub>4</sub> /He = 0.5<br>C <sub>2</sub> H <sub>4</sub>                                                                                           | SiH <sub>4</sub> = 100                    | SiH <sub>4</sub> /C <sub>2</sub> H <sub>4</sub> = 3/7 | 0.18                                              | 10                                    | 0.5                             |

TABLE 3C

| Depth profile |           | Depth profile No. of nitrogen |       |       |       |       |       |       |       |       |        |
|---------------|-----------|-------------------------------|-------|-------|-------|-------|-------|-------|-------|-------|--------|
| No. of boron  | Sample No | 201C                          | 202C  | 203C  | 204C  | 205C  | 206C  | 207C  | 208C  | 209C  | 210C   |
| 101           |           | 1-1C                          | 1-2C  | 1-3C  | 1-4C  | 1-5C  | 1-6C  | 1-7C  | 1-8C  | 1-9C  | 1-10C  |
| 102           |           | 2-1C                          | 2-2C  | 2-3C  | 2-4C  | 2-5C  | 2-6C  | 2-7C  | 2-8C  | 2-9C  | 2-10C  |
| 103           |           | 3-1C                          | 3-2C  | 3-3C  | 3-4C  | 3-5C  | 3-6C  | 3-7C  | 3-8C  | 3-9C  | 3-10C  |
| 104           |           | 4-1C                          | 4-2C  | 4-3C  | 4-4C  | 4-5C  | 4-6C  | 4-7C  | 4-8C  | 4-9C  | 4-10C  |
| 105           |           | 5-1C                          | 5-2C  | 5-3C  | 5-4C  | 5-5C  | 5-6C  | 5-7C  | 5-8C  | 5-9C  | 5-10C  |
| 106           |           | 6-1C                          | 6-2C  | 6-3C  | 6-4C  | 6-5C  | 6-6C  | 6-7C  | 6-8C  | 6-9C  | 6-10C  |
| 107           |           | 7-1C                          | 7-2C  | 7-3C  | 7-4C  | 7-5C  | 7-6C  | 7-7C  | 7-8C  | 7-9C  | 7-10C  |
| 108           |           | 8-1C                          | 8-2C  | 8-3C  | 8-4C  | 8-5C  | 8-6C  | 8-7C  | 8-8C  | 8-9C  | 8-10C  |
| 109           |           | 9-1C                          | 9-2C  | 9-3C  | 9-4C  | 9-5C  | 9-6C  | 9-7C  | 9-8C  | 9-9C  | 9-10C  |
| 110           |           | 10-1C                         | 10-2C | 10-3C | 10-4C | 10-5C | 10-6C | 10-7C | 10-8C | 10-9C | 10-10C |
| 111           |           | 11-1C                         | 11-2C | 11-3C | 11-4C | 11-5C | 11-6C | 11-7C | 11-8C | 11-9C | 11-10C |
| 112           |           | 12-1C                         | 12-2C | 12-3C | 12-4C | 12-5C | 12-6C | 12-7C | 12-8C | 12-9C | 12-10C |
| 113           |           | 13-1C                         | 13-2C | 13-3C | 13-4C | 13-5C | 13-6C | 13-7C | 13-8C | 13-9C | 13-10C |
| 114           |           | 14-1C                         | 14-2C | 14-3C | 14-4C | 14-5C | 14-6C | 14-7C | 14-8C | 14-9C | 14-10C |
| 115           |           | 15-1C                         | 15-2C | 15-3C | 15-4C | 15-5C | 15-6C | 15-7C | 15-8C | 15-9C | 15-10C |
| 116           |           | 16-1C                         | 16-2C | 16-3C | 16-4C | 16-5C | 16-6C | 16-7C | 16-8C | 16-9C | 16-10C |

TABLE 4C

| Depth profile |            | Depth profile No. of nitrogen |       |       |       |       |       |       |       |       |
|---------------|------------|-------------------------------|-------|-------|-------|-------|-------|-------|-------|-------|
| No. of boron  | Sample No. | 401C                          | 402C  | 403C  | 404C  | 405C  | 406C  | 407C  | 408C  | 409C  |
| 301           |            | 21-1C                         | 21-2C | 21-3C | 21-4C | 21-5C | 21-6C | 21-7C | 21-8C | 21-9C |
| 302           |            | 22-1C                         | 22-2C | 22-3C | 22-4C | 22-5C | 22-6C | 22-7C | 22-8C | 22-9C |
| 303           |            | 23-1C                         | 23-2C | 23-3C | 23-4C | 23-5C | 23-6C | 23-7C | 23-8C | 23-9C |
| 304           |            | 24-1C                         | 24-2C | 24-3C | 24-4C | 24-5C | 24-6C | 24-7C | 24-8C | 24-9C |
| 305           |            | 25-1C                         | 25-2C | 25-3C | 25-4C | 25-5C | 25-6C | 25-7C | 25-8C | 25-9C |
| 306           |            | 26-1C                         | 26-2C | 26-3C | 26-4C | 26-5C | 26-6C | 26-7C | 26-8C | 26-9C |
| 307           |            | 27-1C                         | 27-2C | 27-3C | 27-4C | 27-5C | 27-6C | 27-7C | 27-8C | 27-9C |
| 308           |            | 28-1C                         | 28-2C | 28-3C | 28-4C | 28-5C | 28-6C | 28-7C | 28-8C | 28-9C |

TABLE 5C

| Conditions | Gases employed                                                                            | Flow rate (SCCM)                          | Flow rate ratio or Area ratio                                                   | Discharging power (W/cm <sup>2</sup> ) | Layer thickness (μm) |
|------------|-------------------------------------------------------------------------------------------|-------------------------------------------|---------------------------------------------------------------------------------|----------------------------------------|----------------------|
| 1          | Ar                                                                                        | 200                                       | Si wafer:graphite = 1.5:9.5                                                     | 0.3                                    | 0.5                  |
| 2          | Ar                                                                                        | 200                                       | Si wafer: graphite = 0.5:9.5                                                    | 0.3                                    | 0.3                  |
| 3          | Ar                                                                                        | 200                                       | Si wafer:graphite = 6:4                                                         | 0.3                                    | 1.0                  |
| 4          | SiH <sub>4</sub> /He = 1<br>C <sub>2</sub> H <sub>4</sub>                                 | SiH <sub>4</sub> = 150                    | SiH <sub>4</sub> :C <sub>2</sub> H <sub>4</sub> = 0.4:9.6                       | 0.18                                   | 0.3                  |
| 5          | SiH <sub>4</sub> /He = 0.5<br>C <sub>2</sub> H <sub>4</sub>                               | SiH <sub>4</sub> = 100                    | SiH <sub>4</sub> :C <sub>2</sub> H <sub>4</sub> = 5:5                           | 0.18                                   | 1.5                  |
| 6          | SiH <sub>4</sub> /He = 0.5<br>SiF <sub>4</sub> /He = 0.5<br>C <sub>2</sub> H <sub>4</sub> | SiH <sub>4</sub> + SiF <sub>4</sub> = 150 | SiH <sub>4</sub> :SiF <sub>4</sub> :C <sub>2</sub> H <sub>4</sub> = 1.5:1.5:7   | 0.18                                   | 0.5                  |
| 7          | SiH <sub>4</sub> /He = 0.5<br>SiF <sub>4</sub> /He = 0.5<br>C <sub>2</sub> H <sub>4</sub> | SiH <sub>4</sub> + SiF <sub>4</sub> = 150 | SiH <sub>4</sub> :SiF <sub>4</sub> :C <sub>2</sub> H <sub>4</sub> = 0.3:0.1:9.6 | 0.18                                   | 0.3                  |
| 8          | SiH <sub>4</sub> /He = 0.5<br>SiF <sub>4</sub> /He = 0.5<br>C <sub>2</sub> H <sub>4</sub> | SiH <sub>4</sub> + SiF <sub>4</sub> = 150 | SiH <sub>4</sub> :SiF <sub>4</sub> :C <sub>2</sub> H <sub>4</sub> = 3:3:4       | 0.18                                   | 1.5                  |

TABLE 6C

| Layer (III)<br>forming<br>conditions | Sample No./Evaluation |                 |                |
|--------------------------------------|-----------------------|-----------------|----------------|
| 1                                    | 5-5-2-1C<br>○         | 14-10-5-1C<br>○ | 25-3-4-1C<br>○ |
| 2                                    | 5-5-2-2C<br>○         | 14-10-5-2C<br>○ | 25-3-4-2C<br>○ |
| 3                                    | 5-5-2-3C<br>○         | 14-10-5-3C<br>○ | 25-3-4-3C<br>○ |
| 4                                    | 5-5-2-4C<br>○         | 14-10-5-4C<br>○ | 25-3-4-4C<br>○ |
| 5                                    | 5-5-2-5C<br>○         | 14-10-5-5C<br>○ | 25-3-4-5C<br>○ |

TABLE 6C-continued

|    |   |                 |                   |                  |
|----|---|-----------------|-------------------|------------------|
|    | 6 | 5-5-2-6C<br>○ ○ | 14-10-5-6C<br>○ ○ | 25-3-4-6C<br>○ ○ |
|    | 7 | 5-5-2-7C<br>○ ○ | 14-10-5-7C<br>○ ○ | 25-3-4-7C<br>○ ○ |
| 60 | 8 | 5-5-2-8C<br>○ ○ | 14-10-5-8C<br>○ ○ | 25-3-4-8C<br>○ ○ |

Sample No. \_\_\_\_\_  
 Overall image quality evaluation Durability evaluation  
 65: evaluation  
 Evaluation standards:  
 ☺: Excellent  
 ☻: Good  
 ☻: Fair  
 ☻: Poor

TABLE 7C

| Sample No.               | 8-9-4-1C | 8-9-4-2C | 8-9-4-3C | 8-9-4-4C | 8-9-4-5C | 8-9-4-6C | 8-9-4-7C |
|--------------------------|----------|----------|----------|----------|----------|----------|----------|
| Si:C                     | 9:1      | 6.5:3.5  | 4:6      | 2:8      | 1:9      | 0.5:9.5  | 0.2:9.8  |
| Target Area ratio        |          |          |          |          |          |          |          |
| Si:C (Content ratio)     | 9.7:0.3  | 8.8:1.2  | 7.3:2.7  | 4.8:5.2  | 3:7      | 2:8      | 0.8:9.2  |
| Image quality evaluation | Δ        | ○        | ◎        | ◎        | ◎        | Δ        | X        |

◎: Very good

○: Good

Δ: Sufficiently practically usable

X: Image defect formed

TABLE 8C

| Sample No.                                                        | 8-9-4-11C | 8-9-4-12C | 8-9-4-13C | 8-9-4-14C | 8-9-4-15C | 8-9-4-16C | 8-9-4-17C | 8-9-4-18C |
|-------------------------------------------------------------------|-----------|-----------|-----------|-----------|-----------|-----------|-----------|-----------|
| SiH <sub>4</sub> :C <sub>2</sub> H <sub>4</sub> (Flow rate ratio) | 9:1       | 6:4       | 4:6       | 2:8       | 1:9       | 0.5:9.5   | 0.2:9.8   | 0.2:9.8   |
| Si:C (Content ratio)                                              | 9:1       | 7:3       | 5.5:4.5   | 4:6       | 3:7       | 2:8       | 0.8:9.2   | 0.8:9.2   |
| Image quality evaluation                                          | Δ         | ○         | ◎         | ◎         | ◎         | ○         | ○         | X         |

◎: Very good

○: Good

Δ: Sufficiently practically usable

X: Image defect formed

TABLE 9C

| Sample No.                                                                          | 8-9-4-21C | 8-9-4-22C | 8-9-4-23C | 8-9-4-24C | 8-9-4-25C | 8-9-4-26C   | 8-9-4-27C     | 8-9-4-28C   |
|-------------------------------------------------------------------------------------|-----------|-----------|-----------|-----------|-----------|-------------|---------------|-------------|
| SiH <sub>4</sub> :SiF <sub>4</sub> :C <sub>2</sub> H <sub>4</sub> (Flow rate ratio) | 5:4:1     | 3:3.5:3.5 | 2:2:6     | 1:1:8     | 0.4:0.4:9 | 0.2:0.3:9.5 | 0.2:0.15:9.65 | 0.1:0.1:9.8 |
| Si:C (Content ratio)                                                                | 9:1       | 7:3       | 5.5:4.5   | 4:6       | 3:7       | 2:8         | 1.2:8.8       | 0.8:9.2     |
| Image quality evaluation                                                            | Δ         | ○         | ◎         |           | ○         | ○           | ○             | X           |

◎: Very good

○: Good

Δ: Sufficiently practically usable

X: Image defect formed

TABLE 10C

| Sample No. | Thickness of layer (III) (μm) | Results                                                          |
|------------|-------------------------------|------------------------------------------------------------------|
| 8-9-4-31C  | 0.001                         | Image defect liable to occur                                     |
| 8-9-4-32C  | 0.02                          | No image defect formed up to successive copying for 20,000 times |
| 8-9-4-33C  | 0.05                          | Stable up to successive copying for 50,000 times                 |
| 8-9-4-34C  | 1                             | Stable up to successive copying for 200,000 times                |

What we claim is:

1. A photoconductive member comprising a substrate for photoconductive member and a light-receiving layer exhibiting photoconductivity, said light-receiving layer having a layer constitution in which a first layer (I) comprising an amorphous material containing silicon atoms, a second layer (II) comprising an amorphous material containing silicon atoms and germanium atoms and a third layer (III) comprising an amorphous material containing silicon atoms and carbon atoms are successively provided from the substrate side, and the germanium atoms contained in said second layer (II) being distributed ununiformly in the direction of the thickness of said layer and being present in amounts from 1 to

45 9.5 × 10<sup>5</sup> atomic ppm and wherein hydrogen atoms and/or halogen atoms are contained in both the first layer (I) and the second layer (II); and wherein the content of hydrogen and/or halogen atoms (i) in the first layer (the sum of both when both are contained) is 1 to 40 atomic % and (ii) the content of the hydrogen atoms and/or halogen atoms contained in the second layer (ii) (the sum of both when both are contained) is 0.01 to 40 atomic %.

50 2. A photoconductive member according to claim 1, wherein a substance (C) for controlling conductivity is contained in at least one of the first layer (I) and the second layer (II).

3. A photoconductive member according to claim 2, wherein the substance (C) for controlling conductivity is an atom belonging to the group III of the periodic table.

60 4. A photoconductive member according to claim 2, wherein the substance (C) for controlling conductivity is an atom belonging to the group V of the periodic table.

65 5. A photoconductive member according to claim 1, wherein at least one of oxygen atoms and nitrogen atoms are contained in at least one of the first layer (I) and the second layer (II).

6. A photoconductive member according to claim 5, wherein a substance (C) for controlling conductivity is contained in at least one of the first layer (I) and the second layer (II).

7. A photoconductive member according to claim 6, wherein the substance (C) for controlling conductivity is an atom belonging to the group III of the periodic table.

8. A photoconductive member according to claim 6, 10 wherein the substance (C) for controlling conductivity is an atom belonging to the group V of the periodic table.

9. A photoconductive member according to claim 3, 15 wherein the atom belonging to the group III of the periodic table if selected from the group consisting of B, Al, Ga, In and Tl.

10. A photoconductive member according to claim 4, 20 wherein the atom belonging to the group V of the periodic table is selected from the group consisting of P, As, Sb and Bi.

11. A photoconductive member according to claim 5, 25 wherein the content of oxygen atoms and/or nitrogen atoms (the sum of both when both are contained) is 0.001 to 50 atomic %.

12. A photoconductive member according to claim 2, 30 wherein the content of the substance (C) for controlling conductivity in the first layer (I) is 0.001 to  $5 \times 10^4$  atomic ppm.

13. A photoconductive member according to claim 1, 35 wherein the first layer (I) has a thickness of 1000 Å to 50 μm.

14. A photoconductive member according to claim 5, 40 wherein at least one of the oxygen atoms and the nitrogen atoms contained are distributed uniformly in the layer thickness direction.

15. A photoconductive member according to claim 5, 45 wherein at least one of the oxygen atoms and nitrogen atoms contained are distributed ununiformly in the layer thickness direction.

16. A photoconductive member according to claim 1, wherein the second layer (II) has a thickness of 1000 Å to 50 μm.

17. A photoconductive member according to claim 1, 5 wherein the third layer (III) has a thickness of 0.003 to 30 μm.

18. A photoconductive member according to claim 1, wherein the light-receiving layer has a layer region (PN) containing a substance (C) for controlling conductivity.

19. A photoconductive member according to claim 18, wherein the content of the substance (C) for controlling conductivity in the layer region (PN) is 0.001 to  $5 \times 10^4$  atomic ppm.

20. A photoconductive member according to claim 18, wherein the layer region (Z) other than the layer region (PN) contains a substance (C) for controlling conductivity of the polarity different from that of the substance (C) for controlling conductivity contained in the layer region (PN).

21. A photoconductive member according to claim 20, wherein the content of the substance (C) for controlling conductivity contained in the layer region (Z) is 0.001 to 1000 atomic ppm.

22. A photoconductive member according to claim 1, wherein at least one of hydrogen atoms and halogen atoms are contained in the third layer (III).

23. A photoconductive member according to claim 2, wherein a substance for controlling conductivity is contained in at least one of the first layer (I) and the second layer (II).

24. A photoconductive member according to claim 7, wherein the atom belonging to the group III of the periodic table is selected from the group consisting of B, Al, Ga, In and Tl.

25. A photoconductive member according to claim 8, wherein the atom belonging to the group V of the periodic table is selected from the group consisting of P, As, Sb and Bi.

26. A photoconductive member according to claim 6, wherein the content of the substance (C) for controlling conductivity in the first layer (I) is 0.001 to  $5 \times 10^4$  atomic ppm.

\* \* \* \* \*

UNITED STATES PATENT AND TRADEMARK OFFICE  
CERTIFICATE OF CORRECTION

PATENT NO. : 4,598,032

DATED : July 1, 1986

Page 1 of 2

INVENTOR(S) : KEISHI SAITO, ET AL.

It is certified that error appears in the above-identified patent and that said Letters Patent is hereby corrected as shown below:

COLUMN 13

Line 56, "⊖" should read --⊖--.  
Line 61, "⊖" should read --⊖--.

COLUMN 36

TABLE 7A, "3-1-3A" should read --3-1-3A--.  
4:6  
7.3:2.7  
7.3:2.7  
⊖

COLUMN 37

TABLE 10A, "0,001" should read --0.001--.

COLUMN 39

TABLE 6B, "5 5-5-2-5B 14-10-5-5B 25-3-4-5B"  
should read --

5 5-5-2-5B 14-10-5-5B 25-3-4-5B  
⊖ ⊖ ⊖ ⊖ ⊖ ⊖ ⊖ --.

COLUMN 43

TABLE 6C, "1 5-5-2-1C" should read --1 5-5-2-1C--.  
o o

COLUMN 45

TABLE 7C, "Δ o ⊖ ⊖ ⊖ Δ x" should read --Δ ⊖ ⊖ o o Δ x--.

UNITED STATES PATENT AND TRADEMARK OFFICE  
CERTIFICATE OF CORRECTION

PATENT NO. : 4,598,032

DATED : July 1, 1986

Page 2 of 2

INVENTOR(S) : KEISHI SAITO, ET AL.

It is certified that error appears in the above-identified patent and that said Letters Patent is hereby corrected as shown below:

COLUMN 45

TABLE 9C, "Δ o ⊕ o o o x" should read --  
Δ o ⊕ ⊕ ⊕ o o x--.

COLUMN 47

Line 41, "photocnductive" should read --photoconductive--.  
Line 44, "thickens" should read --thickness--.

Signed and Sealed this  
Fourteenth Day of April, 1987

*Attest:*

DONALD J. QUIGG

*Attesting Officer*

*Commissioner of Patents and Trademarks*